



US009492717B2

(12) **United States Patent**  
**Sullivan et al.**

(10) **Patent No.:** **US 9,492,717 B2**  
(45) **Date of Patent:** **Nov. 15, 2016**

(54) **GOLF BALLS HAVING FOAM CENTERS  
WITH NON-UNIFORM CORE STRUCTURES**

(71) Applicant: **Acushnet Company**, Fairhaven, MA (US)

(72) Inventors: **Michael J. Sullivan**, Old Lyme, CT (US); **Mark L. Binette**, Mattapoisett, MA (US); **Brian Comeau**, Berkley, MA (US)

(73) Assignee: **Acushnet Company**, Fairhaven, MA (US)

(\*) Notice: Subject to any disclaimer, the term of this patent is extended or adjusted under 35 U.S.C. 154(b) by 0 days.

(21) Appl. No.: **15/017,888**

(22) Filed: **Feb. 8, 2016**

(65) **Prior Publication Data**

US 2016/0151678 A1 Jun. 2, 2016

**Related U.S. Application Data**

(63) Continuation of application No. 14/184,758, filed on Feb. 20, 2014, now Pat. No. 9,254,422, which is a continuation-in-part of application No. 13/872,354, filed on Apr. 29, 2013, now Pat. No. 9,302,156.

(51) **Int. Cl.**

**A63B 37/06** (2006.01)

**A63B 37/00** (2006.01)

(52) **U.S. Cl.**

CPC ..... **A63B 37/0091** (2013.01); **A63B 37/0032** (2013.01); **A63B 37/0033** (2013.01); **A63B 37/0043** (2013.01); **A63B 37/0044** (2013.01); **A63B 37/0045** (2013.01); **A63B 37/0047** (2013.01); **A63B 37/0058** (2013.01); **A63B 37/0062** (2013.01); **A63B 37/0063** (2013.01); **A63B 37/0064** (2013.01); **A63B 37/0066** (2013.01); **A63B 37/0076** (2013.01); **A63B 37/0092** (2013.01); **A63B 37/0097** (2013.01);

**A63B 37/06** (2013.01); **A63B 37/0005** (2013.01); **A63B 37/0075** (2013.01); **A63B 37/0096** (2013.01); **A63B 2037/065** (2013.01)

(58) **Field of Classification Search**

CPC ..... A63B 37/0058  
USPC ..... 473/376

See application file for complete search history.

(56) **References Cited**

**U.S. PATENT DOCUMENTS**

|                 |         |                    |
|-----------------|---------|--------------------|
| 4,625,964 A     | 12/1986 | Yamada             |
| 5,048,838 A     | 9/1991  | Chikaraishi et al. |
| 5,104,126 A     | 4/1992  | Gentiluomo         |
| 5,688,192 A     | 11/1997 | Aoyama             |
| 5,823,889 A     | 10/1998 | Aoyama             |
| 5,833,553 A     | 11/1998 | Sullivan et al.    |
| 6,293,877 B1    | 9/2001  | Boehm              |
| 6,398,667 B1    | 6/2002  | Lemons             |
| 6,688,991 B2    | 2/2004  | Sullivan et al.    |
| 6,756,436 B2    | 6/2004  | Rajagopalan et al. |
| 6,767,294 B2    | 7/2004  | Nesbitt            |
| 6,773,364 B2    | 8/2004  | Sullivan et al.    |
| 7,022,034 B2    | 4/2006  | Sullivan et al.    |
| 7,708,654 B2    | 5/2010  | Sullivan et al.    |
| 7,901,301 B2    | 3/2011  | Morgan et al.      |
| 8,033,933 B2    | 10/2011 | Sullivan et al.    |
| 8,137,216 B2    | 3/2012  | Sullivan et al.    |
| 8,272,971 B2    | 9/2012  | Tutmark            |
| 2001/0027140 A1 | 10/2001 | Bellinger et al.   |

Primary Examiner — Raeann Gorden

(74) Attorney, Agent, or Firm — Daniel W. Sullivan

(57) **ABSTRACT**

Golf balls having a solid multi-layered core and a cover are provided. The ball contains an inner core made of a foam composition, an intermediate core layer, and surrounding outer core layer. Preferably, foamed polyurethane is used to form the inner core and polybutadiene rubber is used to make the intermediate and outer cores. The specific gravity (density) of the inner core is preferably less than the density of the intermediate core, which is less than the outer core. The outer surface of the inner core preferably has a non-uniform structure and includes projecting members. The ball preferably has a high Moment of Inertia (MOI). The ball includes a single or multi-layered cover surrounding the core assembly.

**17 Claims, 6 Drawing Sheets**





FIG. 2



FIG. 3



FIG. 3

FIG. 4



FIG. 5

FIG. 6



FIG. 7



FIG. 8



FIG. 9



FIG. 10



FIG. 11



FIG. 12



FIG. 13



FIG. 14



FIG. 15

## GOLF BALLS HAVING FOAM CENTERS WITH NON-UNIFORM CORE STRUCTURES

### CROSS-REFERENCE TO RELATED APPLICATIONS

This application is a continuation of co-assigned, U.S. patent application Ser. No. 14/184,785 having a filing date of Feb. 20, 2014, now allowed, which is a continuation-in-part of co-assigned, U.S. patent application Ser. No. 13/872,354 having a filing date of Apr. 29, 2013, now allowed, the entire contents of which are hereby incorporated by reference.

### BACKGROUND OF THE INVENTION

#### 1. Field of the Invention

The present invention generally relates to multi-piece golf balls having a solid core and cover. Particularly, the ball contains an inner core (center) made of a foamed composition and surrounding outer core layer. The inner core is preferably molded from a polyurethane foam material and the outer core is preferably formed from polybutadiene rubber. The outer surface of the inner core preferably has a non-uniform structure and includes projecting members. A single or multi-layered cover may be disposed about the core structure.

#### 2. Brief Review of the Related Art

Multi-piece, solid golf balls having a solid inner core protected by a cover are used today by recreational and professional golfers. The golf balls may have single-layered or multi-layered cores. Normally, the core layers are made of a highly resilient natural or synthetic rubber material such as styrene butadiene, polybutadiene, polyisoprene, or highly neutralized ethylene acid copolymers (HNPs). The covers may be single or multi-layered and made of a durable material such as HNPs, polyamides, polyesters, polyurethanes, and polyureas. Manufacturers of golf balls use different ball constructions (for example, three-piece, four-piece, and five-piece balls) to impart specific properties and features to the balls.

The core is the primary source of resiliency for the golf ball and is often referred to as the "engine" of the ball. The resiliency or coefficient of restitution ("COR") of a golf ball (or golf ball component, particularly a core) means the ratio of a ball's rebound velocity to its initial incoming velocity when the ball is fired out of an air cannon into a rigid plate. The COR for a golf ball is written as a decimal value between zero and one. A golf ball may have different COR values at different initial velocities. The United States Golf Association (USGA) sets limits on the initial velocity of the ball so one objective of golf ball manufacturers is to maximize the COR under these conditions. Balls (or cores) with a high rebound velocity have a relatively high COR value. Such golf balls rebound faster, retain more total energy when struck with a club, and have longer flight distances as opposed to balls with lower COR values. Ball resiliency and COR properties are particularly important for long distance shots. For example, balls having high resiliency and COR values tend to travel a far distance when struck by a driver club from a tee. The spin rate of the ball also is an important property. Balls having a relatively high spin rate are particularly desirable for relatively short distance shots made with irons and wedge clubs. Professional and highly skilled recreational golfers can place a back-spin on such balls more easily. By placing the right amount of spin and touch on the ball, the golfer has better control over shot accuracy and

placement. This is particularly important for approach shots near the green and helps improve scoring performance.

Over the years, golf ball manufacturers have looked at adjusting the density or specific gravity among the multiple layers of the golf ball to control its spin rate. In general, the total weight of a golf ball needs to conform to weight limits set by the United States Golf Association ("USGA"). Although the total weight of the golf ball is mandated, the distribution of weight within the ball can vary. Redistributing the weight or mass of the golf ball either towards the center of the ball or towards the outer surface of the ball changes its flight and spin properties.

For example, the weight can be shifted towards the center of the ball to increase the spin rate of the ball as described in Yamada, U.S. Pat. No. 4,625,964. In the '964 patent, the core composition preferably contains 100 parts by weight of polybutadiene rubber; 10 to 50 parts by weight of zinc acrylate or zinc methacrylate; 10 to 150 parts by weight of zinc oxide; and 1 to 5 parts by weight of peroxide as a cross-linking or curing agent. The inner core has a specific gravity of at least 1.50 in order to make the spin rate of the ball comparable to wound balls. The ball further includes a cover and intermediate layer disposed between the core and cover, wherein the intermediate layer has a lower specific gravity than the core.

Chikaraishi et al., U.S. Pat. No. 5,048,838 discloses a three-piece golf ball containing a two-piece solid core and a cover. The inner core has a diameter in the range of 15-25 mm, a weight of 2-14 grams, a specific gravity of 1.2 to 4.0, and a hardness of 55-80 JISC. The specific gravity of the outer core layer is less than the specific gravity of the inner core by 0.1 to 3.0, less than the specific gravity of the inner core. The inner and outer core layers are formed from rubber compositions.

Gentiluomo, U.S. Pat. No. 5,104,126 discloses a three-piece ball with a dense inner core made of steel, lead, brass, zinc, copper, and a filled elastomer, wherein the core has a specific gravity of at least 1.25. The inner core is encapsulated by a lower density syntactic foam composition, and the core construction is encapsulated by an ionomer cover.

Multi-layered balls containing inner cores made of relatively low-density compositions such as foam also are described in the patent literature. For example, Aoyama, U.S. Pat. Nos. 5,688,192 and 5,823,889 disclose a golf ball containing a core comprising an inner and outer portion, and a cover made of a material such as balata rubber or ethylene acid copolymer ionomer. The core is made by foaming, injecting a compressible material, gasses, blowing agents, or gas-containing microspheres into polybutadiene or other core material. According to the '889 patent, polyurethane compositions may be used. The compressible material, for example, gas-containing compressible cells may be dispersed in a limited part of the core so that the portion containing the compressible material has a specific gravity of greater than 1.00. Alternatively, the compressible material may be dispersed throughout the entire core. In one embodiment, the core comprises an inner and outer portion. In another embodiment, the core comprises inner and outer layers.

Sullivan and Binette, U.S. Pat. No. 5,833,553 discloses a golf ball having core with a coefficient of restitution of at least 0.650 and a cover with a thickness of at least 3.6 mm (0.142 inches) and a Shore D hardness of at least 60. According to the '553 patent, the combination of a soft core with a thick, hard cover results in a ball having better distance. The '553 patent discloses that the core may be formed from a uniform composition or may be a dual or

multi-layer core, and it may be foamed or unfoamed. Polybutadiene rubber, natural rubber, metallocene catalyzed polyolefins, and polyurethanes are described as being suitable materials for making the core.

Sullivan and Ladd, U.S. Pat. No. 6,688,991 discloses a golf ball containing a low specific gravity core and an optional intermediate layer. This sub-assembly is encased within a high specific gravity cover with Shore D hardness in the range of about 40 to about 80. The core is preferably made from a highly neutralized thermoplastic polymer such as ethylene acid copolymer which has been foamed. The cover preferably has high specific gravity fillers dispersed therein.

Nesbitt, U.S. Pat. No. 6,767,294 discloses a golf ball comprising: i) a pressurized foamed inner center formed from a thermoset material, a thermoplastic material, or combinations thereof, a blowing agent and a cross-linking agent and, ii) an outer core layer formed from a second thermoset material, a thermoplastic material, or combinations thereof. Additionally, a barrier resin or film can be applied over the outer core layer to reduce the diffusion of the internal gas and pressure from the nucleus (center and outer core layer). Preferred polymers for the barrier layer have low permeability such as Saran® film (poly(vinylidene chloride), Barex® resin (acrylonitrile-co-methyl acrylate), poly(vinyl alcohol), and PET film (polyethylene terephthalate). The '294 patent does not disclose core layers having different hardness gradients.

Sullivan, Ladd, and Hebert, U.S. Pat. No. 7,708,654 discloses a golf ball having a foamed intermediate layer. Referring to FIG. 1 in the '654 patent, the golf ball includes a core (12), an intermediate layer (14) made of a highly neutralized polymer having a reduced specific gravity (less than 0.95), and a cover (16). According to the '654 patent, the intermediate layer can be an outer core, a mantle layer, or an inner cover. The reduction in specific gravity of the intermediate layer is caused by foaming the composition of the layer and this reduction can be as high as 30%. The '654 patent discloses that other foamed compositions such as foamed polyurethanes and polyureas may be used to form the intermediate layer.

Tutmark, U.S. Pat. No. 8,272,971 is directed to golf balls containing an element that reduces the distance of the ball's flight path. In one embodiment, the ball includes a core and cover. A cavity is formed between core and cover and this may be filled by a foamed polyurethane "middle layer" in order to dampen the ball's flight properties. The foam of the middle layer is relatively light in weight; and the core is relatively heavy and dense. According to the '971 patent, when a golfer strikes the ball with a club, the foam in the middle layer actuates and compresses, thereby absorbing much of the impact from the impact of the ball.

Although some conventional multi-layered core constructions are generally effective in providing high resiliency golf balls, there is a continuing need for improved core constructions in golf balls. Particularly, it would be desirable to have multi-layered core constructions with selective specific gravities and mass densities to provide the ball with good flight distance along with spin control. It further would be desirable to develop core structures, wherein the inner core is made of a low-density material such as a foam composition. The present invention provides core constructions and golf balls having such properties as well as other advantageous features and benefits.

#### SUMMARY OF THE INVENTION

The present invention provides a golf ball comprising an inner core (center), outer core layer, and cover. The multi-

layered core assembly includes: i) an inner core layer comprising a foamed polyurethane composition, and having a center and outer surface and wherein the outer surface contains elements extending outwardly; and ii) an outer core layer comprising a non-foamed thermoset or thermoplastic composition. The inner core preferably has a diameter in the range of about 0.100 to about 1.100 inches; and the outer core layer preferably has a thickness in the range of about 0.200 to about 0.800 inches. Preferably, there is a positive hardness gradient across the core assembly. For example, the ( $H_{inner\ core\ center}$ ) may be in the range of about 10 to about 80 Shore C and the ( $H_{outer\ surface\ of\ OC}$ ) may be in the range of about 65 to about 96 Shore C. A cover having at least one layer is disposed about the multi-layered core assembly.

The inner core has a specific gravity ( $SG_{inner}$ ) and center hardness ( $H_{inner\ core\ center}$ ). In one version, the inner core has a diameter in the range of about 0.20 to about 0.90 inches and a specific gravity in the range of about 0.30 to about 0.95 g/cc. The outer core layer also has a specific gravity ( $SG_{outer\ core}$ ) and outer surface hardness ( $H_{outer\ surface\ of\ OC}$ ). The ( $SG_{outer\ core}$ ) is preferably greater than the ( $SG_{inner}$ ). The outer core layer also may be made from a wide variety of thermoset and thermoplastic materials. For example, a thermoset material such as a polybutadiene, ethylene-propylene, polyisoprene, styrene-butadiene, or butyl rubber composition may be used. Thermoplastic polymers such as partially and highly-neutralized olefin-based acid copolymer ionomer and non-ionomer materials also may be used.

In one preferred embodiment, the projecting members of the outer core are spaced apart and there are gaps between the projections. The projections can be uniformly or randomly spaced apart and can have various shapes and dimensions. In one embodiment, the outer core layer is disposed about the inner core, whereby the outer core material fills the gaps between the projecting members.

The hardness levels of the different layers in the golf ball may vary. For example, in one version, the inner core layer has an outer surface hardness ( $H_{inner\ core\ surface}$ ) and a center hardness ( $H_{inner\ core\ center}$ ), wherein the  $H_{inner\ core\ surface}$  is greater than the  $H_{inner\ core\ center}$  to provide a positive hardness gradient. Meanwhile, the outer core layer has an outer surface hardness ( $H_{outer\ surface\ of\ OC}$ ) and midpoint hardness ( $H_{midpoint\ of\ OC}$ ), wherein the  $H_{outer\ surface\ of\ OC}$  is greater than the ( $H_{midpoint\ of\ OC}$ ), to provide a positive hardness gradient. In another example, the inner core layer has an outer surface hardness ( $H_{inner\ core\ surface}$ ) and a center hardness ( $H_{inner\ core\ center}$ ), wherein the  $H_{inner\ core\ surface}$  is the same or less than the  $H_{inner\ core\ center}$  to provide a zero or negative hardness gradient; while the outer core layer has a positive hardness gradient.

Also, the golf ball may have a variety of cover structures. For example, the cover may have a single layer or multiple layers and be formed from a thermoplastic or thermoset composition. Suitable materials that can be used to form the cover layers include, for example, ethylene acid copolymer ionomers, polyesters, polyamides, polyurethanes, and polyureas.

#### BRIEF DESCRIPTION OF THE DRAWINGS

The novel features that are characteristic of the present invention are set forth in the appended claims. However, the preferred embodiments of the invention, together with further objects and attendant advantages, are best understood by reference to the following detailed description in connection with the accompanying drawings in which:

FIG. 1 is a perspective view of a spherical inner core made of a foamed composition according to the present invention;

FIG. 2 is a cross-sectional view of a three-piece golf ball having a multi-layered core and single-layered cover according to the present invention;

FIG. 3 is a cross-sectional view of a four-piece golf ball having a multi-layered core and dual-layered cover according to the present invention;

FIG. 4 is a cross-sectional view of a three-piece golf ball showing an inner core with projecting members, an outer core, and a cover according to the present invention;

FIG. 5 is a perspective view of the inner core of the golf ball shown in FIG. 4;

FIG. 6 is a plan view along Arrow 4 of the inner core of FIG. 5 according to the present invention;

FIG. 7 is a cross-sectional view of another embodiment of a three-piece ball according to the present invention;

FIG. 8 is a cross-sectional view of another embodiment of a four-piece ball showing an inner core with projecting members, an outer core, an inner cover, and an outer cover according to the present invention;

FIG. 9 is a cross-sectional view of another embodiment of a four-piece ball according to the present invention;

FIG. 10 is a cross-sectional view of another embodiment of a three-piece ball according to the present invention;

FIG. 11 is a cross-sectional view of another embodiment of a three-piece ball according to the present invention;

FIG. 12 is a cross-sectional view of another embodiment of a three-piece ball according to the present invention;

FIG. 13 is a perspective view of another embodiment of the inner core according to the present invention;

FIG. 14 is a perspective view of another embodiment of the inner core according to the present invention; and

FIG. 15 is a perspective view of another embodiment of the inner core according to the present invention.

#### DETAILED DESCRIPTION OF THE INVENTION

##### Golf Ball Constructions

Golf balls having various constructions may be made in accordance with this invention. For example, golf balls having three-piece, four-piece, and five-piece constructions with single or multi-layered cover materials may be made. The term, "layer" as used herein means generally any spherical portion of the golf ball. More particularly, in one version, a three-piece golf ball having a dual-core and cover is made. The dual-core includes an inner core (center) and surrounding outer core layer. In another version, a four-piece golf ball comprising a dual-core and dual-cover (inner cover and outer cover layers) is made. In yet another construction, a four-piece or five-piece golf ball having a multi-layered core; an intermediate (casing) layer, and cover layer(s) may be made. As used herein, the term, "intermediate layer" means a layer of the ball disposed between the core and cover. The intermediate layer also may be referred to as a casing or mantle layer. The diameter and thickness of the different layers along with properties such as hardness and compression may vary depending upon the construction and desired playing performance properties of the golf ball.

In the present invention, the inner core (center) comprises a lightweight foam thermoplastic or thermoset polymer composition. The foam may have an open or closed cellular structure or combinations thereof and the foam may have a structure ranging from a relatively rigid foam to a very flexible foam. Referring to FIG. 1, a foamed inner core (4) having a geometric center (6) and outer skin (8) may be

prepared in accordance with this invention. A wide variety of thermoplastic and thermoset materials may be used in forming the foam composition as described further below. Referring to FIG. 2, one version of a golf ball that can be made in accordance with this invention is generally indicated at (10). The ball (10) contains a multi-layered core (12) having an inner core (center) (12a) and outer core layer (12b) surrounded by a single-layered cover (14). As shown in FIG. 3, in another version, the golf ball (16) contains a dual-layered core having a center (18) and outer core layer (20) surrounded by an inner cover (22). An outer cover (24) is disposed about the inner cover (22).

In one embodiment, the inner core (18) is relatively small in volume and generally has a diameter within a range of about 0.10 to about 1.10 inches. More particularly, the inner core (18) preferably has a diameter size with a lower limit of about 0.15 or 0.25 or 0.35 or 0.45 or 0.50 or 0.55 inches and an upper limit of about 0.60 or 0.70 or 0.80 or 0.90 inches. In one preferred version, the diameter of the inner core (18) is in the range of about 0.15 to about 0.80 inches, more preferably about 0.30 to about 0.75 inches. In a particularly preferred version, the diameter of the inner core (18) is about 0.5 inches. Meanwhile, the outer core layer (20) generally has a thickness within a range of about 0.10 to about 0.85 inches and preferably has a lower limit of 0.10 or 0.15 or 0.20 or 0.25 or 0.30 or 0.32 or 0.35 or 0.40 or 0.45 inches and an upper limit of 0.50 or 0.52 or 0.60 or 0.65 or 0.68 or 0.70 or 0.75 or 0.78 or 0.80 or 0.85 inches. In one preferred version, the outer core layer (20) has a thickness in the range of about 0.40 to about 0.70 inches, more preferably about 0.50 to about 0.65 inches. In a particularly preferred version, the thickness of the outer core (20) is about 0.51 inches; and the total diameter of the inner core/outer core sub-assembly is about 1.53 inches.

Golf balls made in accordance with this invention can be of any size, although the USGA requires that golf balls used in competition have a diameter of at least 1.68 inches. For play outside of United States Golf Association (USGA) rules, the golf balls can be of a smaller size. Normally, golf balls are manufactured in accordance with USGA requirements and have a diameter in the range of about 1.68 to about 1.80 inches. In general, the multi-layer core structure has an overall diameter within a range having a lower limit of about 1.00 or 1.20 or 1.30 or 1.40 inches and an upper limit of about 1.58 or 1.60 or 1.62 or 1.66 inches, and more preferably in the range of about 1.3 to 1.65 inches. In one embodiment, the diameter of the core subassembly is in the range of about 1.45 to about 1.62 inches.

As discussed further below, various compositions may be used to make the dual-core structures of the golf balls of this invention. Different compositions are used and the specific gravity and weight of the core layers are adjusted as needed.

The specific gravity (density) of the respective core layers is an important property, because they affect the Moment of Inertia (MOI) of the ball as discussed further below. The foamed inner core preferably has a specific gravity of about 0.25 to about 1.25 g/cc. That is, the density of the inner core (as measured at any point of the inner core structure) is preferably within the range of about 0.25 to about 1.25 g/cc. By the term, "specific gravity of the inner core" ("SG<sub>inner</sub>"), it is generally meant the specific gravity of the inner core as measured at any point of the inner core structure. It should be understood, however, that the specific gravity values, as taken at different points of the inner core structure, may vary. For example, the foamed inner core may have a "positive" density gradient (that is, the outer surface (skin) of the inner core may have a density greater than the geometric center of

the inner core.) In one preferred version, the specific gravity of the geometric center of the inner core ( $SG_{center\ of\ inner\ core}$ ) is less than 1.00 g/cc and more preferably 0.90 g/cc or less.

More particularly, in one version, the ( $SG_{center\ of\ inner\ core}$ ) is in the range of about 0.10 to about 0.90 g/cc. For example, the ( $SG_{center\ of\ inner\ core}$ ) may be within a range having a lower limit of about 0.10 or 0.15 of 0.20 or 0.24 or 0.30 or 0.35 or 0.37 or 0.40 or 0.42 or 0.45 or 0.47 or 0.50 and an upper limit of about 0.60 or 0.65 or 0.70 or 0.74 or 0.78 or 0.80, or 0.82 or 0.84 or 0.85 or 0.88 or 0.90 g/cc. Meanwhile, the specific gravity of the outer surface (skin) of the inner core ( $SG_{skin\ of\ inner\ core}$ ), in one preferred version, is greater than about 0.90 g/cc and more preferably greater than 1.00 g/cc. For example, the ( $SG_{skin\ of\ inner\ core}$ ) may fall within the range of about 0.90 to about 2.00. More particularly, in one version, the ( $SG_{skin\ of\ inner\ core}$ ) may have a specific gravity with a lower limit of about 0.90 or 0.92 or 0.95 or 0.98 or 1.00 or 1.02 or 1.06 or 1.10 or 1.12 or 1.15 or 1.18 and an upper limit of about 1.20 or 1.24 or 1.30 or 1.32 or 1.35 or 1.38 or 1.40 or 1.44 or 1.50 or 1.60 or 1.65 or 1.70 or 1.76 or 1.80 or 1.90 or 1.92 or 2.00. In other instances, the outer skin may have a specific gravity of less than 0.90 g/cc. For example, the specific gravity of the outer skin ( $SG_{skin\ of\ inner\ core}$ ) may be about 0.75 or 0.80 or 0.82 or 0.85 or 0.88 g/cc. In such instances, wherein both the ( $SG_{center\ of\ inner\ core}$ ) and ( $SG_{skin\ of\ inner\ core}$ ) are less than 0.90 g/cc, it is still preferred that the ( $SG_{center\ of\ inner\ core}$ ) is less than the ( $SG_{skin\ of\ inner\ core}$ ).

Meanwhile, the outer core layer preferably has a relatively high specific gravity. Thus, the specific gravity of the inner core layer ( $SG_{inner}$ ) is preferably less than the specific gravity of the outer core layer ( $SG_{outer}$ ). By the term, "specific gravity of the outer core layer" ("SG<sub>outer</sub>"), it is generally meant the specific gravity of the outer core layer as measured at any point of the outer core layer. The specific gravity values at different points in the outer core layer may vary. That is, there may be specific gravity gradients in the outer core layer similar to the inner core. For example, the outer core layer may have a specific gravity within a range having a lower limit of about 0.50 or 0.60 or 0.70 or 0.75 or 0.85 or 0.95 or 1.00 or 1.10 or 1.25 or 1.30 or 1.36 or 1.40 or 1.42 or 1.48 or 1.50 or 1.60 or 1.66 or 1.75 or 2.00 and an upper limit of 2.50 or 2.60 or 2.80 or 2.90 or 3.00 or 3.10 or 3.25 or 3.50 or 3.60 or 3.80 or 4.00, 4.25 or 5.00 or 5.10 or 5.20 or 5.30 or 5.40 or 6.00 or 6.20 or 6.25 or 6.30 or 6.40 or 6.50 or 7.00 or 7.10 or 7.25 or 7.50 or 7.60 or 7.65 or 7.80 or 8.00 or 8.20 or 8.50 or 9.00 or 9.75 or 10.00 g/cc.

#### Core Structure—Geometric Projections and Thickness

As shown in FIGS. 1-3, in some embodiments, the inner core has a substantially spherical shape and uniform thickness. In this version, the inner core includes a geometric center and outer surface that is substantially free of any projections or extending members. In these embodiments, the inner core has a substantially uniform thickness and the outer surface of the inner core has a substantially smooth surface.

Referring to FIGS. 4 to 15, in other embodiments, the inner core structure has a non-uniform thickness and/or contains projecting members. These extending members on the outer surface of the core may be arranged in any suitable geometric pattern. For example, the extending members may be arranged in a grid or lattice; or a series of rows and raised columns. These extending members may be in the form of ridges, bumps, nubs, hooks, juts, ribs, segments, brambles, spines, projections, points, protrusions, and the like. The projections on the outer surface may have any suitable shape and dimensions, and they may be arranged randomly or in

a geometric order. For example, the projections may have a circular, oval, triangular, square, rectangular, pentagonal, hexagonal, heptagonal, or octagonal. Conical-shaped projections also may be used. The projections may be arranged in linear or non-linear patterns such as arcs and curves. The projections may be configured so there are gaps or channels located between them. The outer surface of inner core also may contain depressions, cavities, and the like. These recessed areas can be arranged so the outer surface has a series of peaks and valleys.

Suitable projecting members and various designs, patterns, and outlays of the members are disclosed in Sullivan et al., U.S. Pat. Nos. 8,137,216 and 8,033,933; Morgan et al., U.S. Pat. No. 7,901,301; Sullivan et al., U.S. Pat. Nos. 7,022,034 and 6,773,364; Rajagopalan et al., U.S. Pat. No. 6,939,907; and Boehm, U.S. Pat. No. 6,293,877, the disclosures of which are hereby incorporated by reference.

More particularly, referring to FIGS. 4-6, the golf ball (25) includes an inner core (26) an outer core (27, 28), a cover (29) (shown without dimples). The inner core (26) includes a three-dimensional outer surface (30), a center C, a central portion (32), and a plurality of projections (35). The central portion (32) and projections (35) are integrally formed, so that the inner core is a single piece. The outer core includes a first section (27) and a second section (28). The first section (27) fills the gaps (40) around the projections (35), and is disposed between the side walls (55) of adjacent projections (35). It is preferred that the diameter of the core which includes the inner core and the outer core is between about 1.00 inches and about 1.64 inches for a ball having a diameter of 1.68 inches. The second section (28) fills the recesses (50) of each projection (35) and is disposed between the side walls (55) of a single projection (35). The outer core sections (27, 28) are formed so that the outer core terminates flush with the free end (45) of each projection (35). The outer core has a substantially spherical outer surface. The cover (29) is formed about the inner core (26) and the outer core sections (27, 28) so that both the inner and outer cores abut the cover. The formation of the golf ball starts with forming the inner core (26). The inner core (26), outer core sections (27, 28), and the cover (29) are formed by compression molding, injection molding, or casting.

As shown in FIG. 5, each recess (50) is formed by three integral side walls (55). Each of the side walls (55) is shaped like a flat quarter circle. The quarter circle includes two straight edges (60) joined by a curved edge (65). In each projection (35), each of the side walls (55) is joined at the straight edges (60). The curved edges (65) of each of the projections allow the inner core to have a spherical shape. With reference to a three-dimensional Cartesian Coordinate system, there are perpendicular x, y, and z axes, respectively that form eight octants. There are eight projections (35) with one in each octant of the coordinate system, so that each of the projections (35) forms an octant of the skeletal sphere. Thus, the inner core is symmetrical. The gaps (40) define three perpendicular concentric rings  $70_x$ ,  $70_y$ , and  $70_z$ . The subscript for the reference number (70) designates the central axis of the ring about which the ring circumscribes.

In FIG. 6, the outer surface (33) of the inner core (26) is defined by radial distances from the center C. At least two of the radial distances about the outer surface are different. The central portion (32) has a radius, designated by the arrow  $r_{cp}$ , that extends from the core center C to the outer surface of the central portion. The central portion 32 is solid in this embodiment.

As shown in FIGS. 5 and 6, each of the projections (35) extends radially outwardly from the central portion (32), and

the projections (35) are spaced from one another to define gaps (40) there between. The projections (35) are shaped so that the inner core (26) is substantially spherically symmetrical. Each projection (35) has an enlarged free end (45) and a substantially conical shape. Each free end (45) includes an open recess (50). Each projection (35) has a radius, designated by the arrow  $r_p$ , that extends from the core center C to the outer surface (33) at the free end (45). The projection radii  $r_p$  differ from the central portion radius  $r_{cp}$ .

In FIG. 7, another embodiment of the golf ball (505) is shown. The golf ball (505) includes an outer core with a first section (515) and a second section (520). The first section (515) and second section (520) are formed of two materials with different material properties. Referring to FIG. 8, another embodiment of a golf ball (605) is shown. The golf ball (605) includes an intermediate (casing) layer (612) disposed between the cover (625) and the core structure (inner core 610 and outer cores 615 and 620). The intermediate layer (612) is formed of either outer core material, cover material, or a different material. The first section (615) and second section (620) of the outer core may be formed of materials with the same material properties. However, in another embodiment, the outer core sections (615, 620) are formed of different materials. The intermediate layer (612) covers the inner core (610), outer core (615 and 620), and forms a continuous layer beneath the cover (625). Another embodiment of a golf ball (705) is shown in FIG. 9. The golf ball (705) includes an intermediate (casing) layer (712) disposed between the cover (725) and the core structure (inner core 710 and outer cores 715 and 720). The intermediate layer (712) is formed of either outer core material, cover material or a different material. The first section (715) and second section (720) of the outer core are formed of materials with different material properties. The intermediate layer (712) covers the inner core (710), outer core (715 and 720), and forms a continuous layer beneath the cover (725). In FIG. 10, another embodiment of the golf ball (805) is shown. The golf ball (805) includes an outer core with a multi-material first section (815a and 815b) disposed within the gaps (840). The different portions (815a, 815b) of the first section of the outer core are formed of two materials with different material properties. In other embodiments, additional layers may be added to those mentioned above or the existing layers may be formed by multiple materials.

Turning to FIG. 11, the golf ball (905) includes an inner core (910) including a central portion (930) and plurality of outwardly radially extending projections (935). The inner core (910) includes a hollow central portion (930) that defines a chamber (990) therein. The outer core is formed from a first section (915) disposed within the gaps (940), and a second section (920) disposed within the recesses (95). The first and second sections (915, 920) may be formed of a material with the same material properties. The cover section (925) surrounds the outer core (915, 920). The hollow central portion (930) reduces the volume of the inner core (910) material. In other embodiment, the central portion (930) may include a fluid.

Referring to FIG. 12, the golf ball (1005) includes an inner core (1010) and outer core (1015, 1020). The inner core (1010) includes a central portion (1030) and plurality of outwardly radially extending projections (1035). The central portion (1030) is hollow and surrounds a fluid-filled center (1095). The fluid-filled center (1095) is formed of an envelope (1096) containing a fluid (1097). The outer core is formed from a first section (1015) disposed within the gaps (1040), and a second section (1020) disposed within the recesses (1050). The first and second sections (1020, 1050)

may be formed of a material with the same material properties. The cover material (1025) surrounds the inner and outer cores. In FIG. 12, the inner core (1020) includes a center (1095). When the center (1095) is fluid-filled, the center (1095) is formed first and then the inner core (1020) is molded around the center. Conventional molding techniques can be used for this operation. Then, the outer core (1015, 1020) and cover (1025) are formed thereon, as discussed above.

10 Another embodiment of an inner core (2010) is shown in FIG. 13. The inner core (2010) includes a spherical central portion (2030) having an outer surface (2031), and a plurality of projections (2035) extending radially outwardly from the central portion (2030). The projections (2035) include a base (2036) adjacent the outer surface (2031) and a pointed free-end (2038). The projections (2035) are substantially conical and taper from the base (2036) to the pointed free-end (2038). It is preferred that the bases cover greater than about 15% of the outer surface. More preferably, the bases should cover greater than about 50% of the outer surface. Most preferably, the bases should be circular in shape and cover greater than about 80% of the outer surface and less than about 85%. As a result, the projections (2035) are spaced from one another and the area of the outer surface (2031) between each projection base (2036) is less than the area of each base. The projections (2035) are conical and configured so that the free ends (2038) of the projections form a spheroid. The base can have other shapes, such as polygons. Examples of polygon shapes that can be used for the base are triangles, pentagons, and hexagons. In addition, instead of the projections having a circular cross-section they can have other cross-sectional shapes such as square.

35 The projections further include a base diameter, designated by the letter d, and a projection height, designated by the letter h. It is preferred that the base diameter d is greater than or equal to the projection height h. This allows an included angle  $\alpha$  between two diametrically opposed sides of the projection, designated L1 and L2, to be about 60° or 40 more. More preferably, the angle  $\alpha$  is about 90° or more and most preferably the angle  $\alpha$  is about 135°. This allows a simple mold to be used from which the core can be extracted. To form a golf ball with inner core (2010), an outer core, as discussed above, is disposed around the inner core (2010) so that the outer core material is disposed within the gaps (2040) and the outer surface of the outer core is substantially spherical. The materials for the inner and outer cores are as discussed above. Then, the cover is formed thereon. The outer surface of the inner core has non-uniform radial distances from the center to various locations on the outer surface due to the conical projections (2035).

55 In FIGS. 14-15, different inner core (3010, 4010) structures are shown. In FIG. 14, the outer surface (3020) of the inner core includes a plurality of projections (3035) formed so that gaps (3040) are formed surrounding each projection and between projections. Each projection includes a maximum length, which is the longest length of the projection, designated L. Each projection also includes a maximum width, which is the widest width of the projection, designated W. The surface of the projection is curved along the length L and width W. A substantial number of projections have the maximum length greater than the maximum width so that the projections are elongated. To form a golf ball, an outer core, as discussed above, is disposed around the inner core (3010) so that the outer core material is disposed within the gaps. The outer core material forms a substantially spherical surface. The materials for the inner and outer cores

are as discussed above. Then, a cover is formed thereon. The outer surface of the inner core has non-uniform radial distances from the center due to the projections and the indentations. In this embodiment, in order to form the outer surface of this inner core, the first, second and third surfaces are formed by rotation of a wave form about first, second and third axes, respectively. These axii are the x-, y- and z-axii in a Cartesian Coordinate System. The wave form used is sine wave. However, other wave forms can be used including, but not limited to, cosine or saw-tooth wave forms.

In FIG. 15, the outer surface (4020) of the inner core (4010) includes a plurality of projections (4035) formed so that gaps (4040) are formed surrounding each projection and between projections. Each projection includes a maximum length, which is the longest length of the projection, designated L. Each projection also includes a maximum width, which is the widest width of the projection, designated W. The surface of the projection is curved along the length L and width W. A substantial number of projections have the maximum length greater than the maximum width so that the projections are elongated. In this embodiment, in order to form the outer surface of this inner core, the first, second, and third surfaces are formed as discussed above, and a fourth surface that is formed by rotating the wave form about a fourth axis that is about 45° from the first and second axii. The surface of the inner core (4020) is formed by the intersection of the first, second, third and fourth surfaces. Any number of surfaces greater than three can be used to create different outer surface geometries for the inner core. Furthermore, different axii can also be used.

#### Hardness of the Inner Core

As shown in FIG. 1, a foamed inner core (4) having a geometric center (6) and outer skin (8) may be prepared per the molding method discussed above. The outer skin (8) is generally a non-foamed region that forms the outer surface of the core structure. The resulting inner core preferably has a diameter within a range of about 0.100 to about 1.100 inches. For example, the inner core may have a diameter within a range of about 0.250 to about 1.000 inches. In another example, the inner core may have a diameter within a range of about 0.300 to about 0.800 inches. More particularly, the inner core preferably has a diameter size with a lower limit of about 0.10 or 0.12 or 0.15 or 0.17 or 0.25 or 0.30 or 0.35 or 0.38 or 0.45 or 0.50 or 0.52 or 0.55 inches and an upper limit of about 0.60 or 0.63 or 0.65 or 0.70 or 0.74 or 0.80 or 0.86 or 0.90 or 0.95 or 1.00 or 1.02 or 1.10 inches. The outer skin (8) of the inner core is relatively thin preferably having a thickness of less than about 0.020 inches and more preferably less than 0.010 inches. In one preferred embodiment, the foamed core has a “positive” hardness gradient (that is, the outer skin of the inner core is harder than its geometric center.)

For example, the geometric center hardness of the inner core ( $H_{inner\ core\ center}$ ), as measured in Shore C units, may be about 10 Shore C or greater and preferably has a lower limit of about 10 or 13 or 16 or 20 or 25 or 30 or 32 or 34 or 36 or 40 Shore C and an upper limit of about 42 or 44 or 48 or 50 or 52 or 56 or 60 or 62 or 65 or 68 or 70 or 74 or 78 or 80 or 84 or 90 Shore C. In one preferred version, the geometric center hardness of the inner core ( $H_{inner\ core\ center}$ ) is about 40 Shore C.

When a flexible, relatively soft foam is used, the ( $H_{inner\ core\ center}$ ) of the foam may have a Shore A hardness of about 10 or greater, and preferably has a lower limit of 15, 18, 20, 25, 28, 30, 35, 38, or 40 Shore A hardness and an upper limit of about 45 or 48, or 50, 54, 58, 60, 65, 70, 80,

85, or 90 Shore A hardness. In one preferred embodiment, the ( $H_{inner\ core\ center}$ ) of the foam is about 55 Shore A.

The ( $H_{inner\ core\ center}$ ), as measured in Shore D units, is about 15 Shore D or greater and more preferably within a range having a lower limit of about 15 or 18 or 20 or 22 or 25 or 28 or 30 or 32 or 36 or 40 or 44 Shore D and an upper limit of about 45 or 48 or 50 or 52 or 55 or 58 or 60 or 62 or 64 or 66 or 70 or 72 or 74 or 78 or 80 or 82 or 84 or 88 or 90 Shore D.

Meanwhile, the outer surface hardness of the inner core ( $H_{inner\ core\ surface}$ ), as measured in Shore C, is preferably about 20 Shore C or greater and may have, for example, a lower limit of about 10 or 14 or 17 or 20 or 22 or 24 or 28 or 30 or 32 or 35 or 36 or 40 or 42 or 44 or 48 or 50 Shore C and an upper limit of about 52 or 55 or 58 or 60 or 62 or 64 or 66 or 70 or 74 or 78 or 80 or 86 or 88 or 90 or 92 or 95 Shore C. When a flexible, relatively soft foam is used, the ( $H_{inner\ core\ surface}$ ) of the foam may have a Shore A hardness of about 12 or greater, and preferably has a lower limit of 12, 16, 20, 24, 26, 28, 30, 34, 40, 42, 46, or 50 Shore A hardness and an upper limit of about 52, 55, 58, 60, 62, 66, 70, 74, 78, 80, 84, 88, 90, or 92 Shore A hardness. In one preferred embodiment, the ( $H_{inner\ core\ surface}$ ) is about 60 Shore A. The ( $H_{inner\ core\ surface}$ ), as measured in Shore D units, preferably has a lower limit of about 25 or 28 or 30 or 32 or 36 or 40 or 44 Shore D and an upper limit of about 45 or 48 or 50 or 52 or 55 or 58 or 60 or 62 or 64 or 66 or 70 or 74 or 78 or 80 or 82 or 84 or 88 or 90 or 94 or 96 Shore D.

#### Density of the Inner Core

The foamed inner core preferably has a specific gravity of about 0.20 to about 1.00 g/cc. That is, the density of the inner core (as measured at any point of the inner core structure) is preferably within the range of about 0.20 to about 1.00 g/cc. By the term, “specific gravity of the inner core” (“ $SG_{inner}$ ”), it is generally meant the specific gravity of the inner core as measured at any point of the inner core structure. It should be understood, however, that the specific gravity values, as taken at different particular points of the inner core structure, may vary. For example, the foamed inner core may have a “positive” density gradient (that is, the outer surface (skin) of the inner core may have a density greater than the geometric center of the inner core.) In one preferred version, the specific gravity of the geometric center of the inner core ( $SG_{center\ of\ inner\ core}$ ) is less than 0.80 g/cc and more preferably less than 0.70 g/cc. More particularly, in one version, the ( $SG_{center\ of\ inner\ core}$ ) is in the range of about 0.10 to about 0.06 g/cc. For example, the ( $SG_{center\ of\ inner\ core}$ ) may be within a range having a lower limit of about 0.10 or 0.15 of 0.20 or 0.24 or 0.30 or 0.35 or 0.37 or 0.40 or 0.42 or 0.45 or 0.47 or 0.50 and an upper limit of about 0.60 or 0.65 or 0.70 or 0.74 or 0.78 or 0.80, or 0.82 or 0.84 or 0.85 or 0.88 or 0.90 g/cc. Meanwhile, the specific gravity of the outer surface (skin) of the inner core ( $SG_{skin\ of\ inner\ core}$ ), in one preferred version, is greater than about 0.90 g/cc and more preferably greater than 1.00 g/cc. For example, the ( $SG_{skin\ of\ inner\ core}$ ) may fall within the range of about 0.90 to about 1.25 g/cc. More particularly, in one version, the ( $SG_{skin\ of\ inner\ core}$ ) may have a specific gravity with a lower limit of about 0.90 or 0.92 or 0.95 or 0.98 or 1.00 or 1.02 or 1.06 or 1.10 g/cc and an upper limit of about 1.12 or 1.15 or 1.18 or 1.20 or 1.24 or 1.30 or 1.32 or 1.35 g/cc. In other instances, the outer skin may have a specific gravity of less than 0.90 g/cc. For example, the specific gravity of the outer skin ( $SG_{skin\ of\ inner\ core}$ ) may be about 0.75 or 0.80 or 0.82 or 0.85 or 0.88 g/cc. In such instances, wherein both the ( $SG_{center\ of\ inner\ core}$ ) and ( $SG_{skin\ of\ inner\ core}$ ) are less than

0.90 g/cc, it is still preferred that the (SG<sub>center of inner core</sub>) be less than the (SG<sub>skin of inner core</sub>).

Core Structure—Hardness

The hardness of the core sub-assembly (inner core and outer core layer) also is an important property. In general, cores with relatively high hardness values have higher compression and tend to have good durability and resiliency. However, some high compression balls are stiff and this may have a detrimental effect on shot control and placement. Thus, the optimum balance of hardness in the core sub-assembly needs to be attained. As discussed above, the inner core is preferably formed from a foamed thermoplastic or thermoset composition and more preferably foamed polyurethanes. And, the outer core layer is formed preferably from a non-foamed thermoset composition such as polybutadiene rubber. Dual-layered core structures containing layers with various thickness and volume levels may be made in accordance with this invention.

In one preferred golf ball, the inner core (center) has a “positive” hardness gradient (that is, the outer surface of the inner core is harder than its geometric center); and the outer core layer has a “positive” hardness gradient (that is, the outer surface of the outer core layer is harder than the inner surface of the outer core layer.) In such cases where both the inner core and outer core layer each has a “positive” hardness gradient, the outer surface hardness of the outer core layer is preferably greater than the hardness of the geometric center of the inner core. In one preferred version, the positive hardness gradient of the inner core is in the range of about 2 to about 40 Shore C units and even more preferably about 10 to about 25 Shore C units; while the positive hardness gradient of the outer core is in the range of about 2 to about 20 Shore C and even more preferably about 3 to about 10 Shore C.

In an alternative version, the inner core may have a positive hardness gradient; and the outer core layer may have a “zero” hardness gradient (that is, the hardness values of the outer surface of the outer core layer and the inner surface of the outer core layer are substantially the same) or a “negative” hardness gradient (that is, the outer surface of the outer core layer is softer than the inner surface of the outer core layer.) For example, in one version, the inner core has a positive hardness gradient; and the outer core layer has a negative hardness gradient in the range of about 2 to about 25 Shore C. In a second alternative version, the inner core may have a zero or negative hardness gradient; and the outer core layer may have a positive hardness gradient. Still yet, in another embodiment, both the inner core and outer core layers have zero or negative hardness gradients.

In general, hardness gradients are further described in Bulpitt et al., U.S. Pat. Nos. 7,537,529 and 7,410,429, the disclosures of which are hereby incorporated by reference. Methods for measuring the hardness of the inner core and outer core layers along with other layers in the golf ball and determining the hardness gradients of the various layers are described in further detail below. The core layers have positive, negative, or zero hardness gradients defined by hardness measurements made at the outer surface of the inner core (or outer surface of the outer core layer) and radially inward towards the center of the inner core (or inner surface of the outer core layer). These measurements are made typically at 2-mm increments as described in the test methods below. In general, the hardness gradient is determined by subtracting the hardness value at the innermost portion of the component being measured (for example, the center of the inner core or inner surface of the outer core layer) from the hardness value at the outer surface of the

component being measured (for example, the outer surface of the inner core or outer surface of the outer core layer).

Positive Hardness Gradient.

For example, if the hardness value of the outer surface of the inner core is greater than the hardness value of the inner core’s geometric center (that is, the inner core has a surface harder than its geometric center), the hardness gradient will be deemed “positive” (a larger number minus a smaller number equals a positive number.) For example, if the outer surface of the inner core has a hardness of 67 Shore C and the geometric center of the inner core has a hardness of 60 Shore C, then the inner core has a positive hardness gradient of 7. Likewise, if the outer surface of the outer core layer has a greater hardness value than the inner surface of the outer core layer, the given outer core layer will be considered to have a positive hardness gradient.

Negative Hardness Gradient.

On the other hand, if the hardness value of the outer surface of the inner core is less than the hardness value of the inner core’s geometric center (that is, the inner core has a surface softer than its geometric center), the hardness gradient will be deemed “negative.” For example, if the outer surface of the inner core has a hardness of 68 Shore C and the geometric center of the inner core has a hardness of 70 Shore C, then the inner core has a negative hardness gradient of 2. Likewise, if the outer surface of the outer core layer has a lesser hardness value than the inner surface of the outer core layer, the given outer core layer will be considered to have a negative hardness gradient.

Zero Hardness Gradient.

In another example, if the hardness value of the outer surface of the inner core is substantially the same as the hardness value of the inner core’s geometric center (that is, the surface of the inner core has about the same hardness as the geometric center), the hardness gradient will be deemed “zero.” For example, if the outer surface of the inner core and the geometric center of the inner core each has a hardness of 65 Shore C, then the inner core has a zero hardness gradient. Likewise, if the outer surface of the outer core layer has a hardness value approximately the same as the inner surface of the outer core layer, the outer core layer will be considered to have a zero hardness gradient.

More particularly, the term, “positive hardness gradient” as used herein means a hardness gradient of positive 3 Shore C or greater, preferably 7 Shore C or greater, more preferably 10 Shore C, and even more preferably 20 Shore C or greater. The term, “zero hardness gradient” as used herein means a hardness gradient of less than 3 Shore C, preferably less than 1 Shore C and may have a value of zero or negative 1 to negative 10 Shore C. The term, “negative hardness gradient” as used herein means a hardness value of less than zero, for example, negative 3, negative 5, negative 7, negative 10, negative 15, or negative 20 or negative 25. The terms, “zero hardness gradient” and “negative hardness gradient” may be used herein interchangeably to refer to hardness gradients of negative 1 to negative 10.

The inner core preferably has a geometric center hardness (H<sub>inner core center</sub>) of about 5 Shore D or greater. For example, the (H<sub>inner core center</sub>) may be in the range of about 5 to about 88 Shore D and more particularly within a range having a lower limit of about 5 or 10 or 18 or 20 or 26 or 30 or 34 or 36 or 38 or 42 or 48 or 50 or 52 Shore D and an upper limit of about 54 or 56 or 58 or 60 or 62 or 64 or 68 or 70 or 74 or 76 or 80 or 82 or 84 or 88 Shore D. In another example, the center hardness of the inner core (H<sub>inner core center</sub>), as measured in Shore C units, is preferably about 10 Shore C or greater; for example, the H<sub>inner core center</sub>

may have a lower limit of about 10 or 14 or 16 or 20 or 23 or 24 or 28 or 31 or 34 or 37 or 40 or 44 Shore C and an upper limit of about 46 or 48 or 50 or 51 or 53 or 55 or 58 or 61 or 62 or 65 or 68 or 71 or 74 or 76 or 78 or 79 or 80 or 84 or 90 Shore C. Concerning the outer surface hardness of the inner core ( $H_{inner\ core\ surface}$ ), this hardness is preferably about 12 Shore D or greater; for example, the  $H_{inner\ core\ surface}$  may fall within a range having a lower limit of about 12 or 15 or 18 or 20 or 22 or 26 or 30 or 34 or 36 or 38 or 42 or 48 or 50 or 52 Shore D and an upper limit of about 54 or 56 or 58 or 60 or 62 or 70 or 72 or 75 or 78 or 80 or 82 or 84 or 86 or 90 Shore D. In one version, the outer surface hardness of the inner core ( $H_{inner\ core\ surface}$ ), as measured in Shore C units, has a lower limit of about 13 or 15 or 18 or 20 or 22 or 24 or 27 or 28 or 30 or 32 or 34 or 38 or 44 or 47 or 48 Shore C and an upper limit of about 50 or 54 or 56 or 61 or 65 or 66 or 68 or 70 or 73 or 76 or 78 or 80 or 84 or 86 or 88 or 90 or 92 Shore C. In another version, the geometric center hardness ( $H_{inner\ core\ center}$ ) is in the range of about 10 Shore C to about 50 Shore C; and the outer surface hardness of the inner core ( $H_{inner\ core\ surface}$ ) is in the range of about 5 Shore C to about 50 Shore C.

On the other hand, the outer core layer preferably has an outer surface hardness ( $H_{outer\ surface\ of\ OC}$ ) of about 40 Shore D or greater, and more preferably within a range having a lower limit of about 40 or 42 or 44 or 46 or 48 or 50 or 52 and an upper limit of about 54 or 56 or 58 or 60 or 62 or 64 or 70 or 74 or 78 or 80 or 82 or 85 or 87 or 88 or 90 Shore D. The outer surface hardness of the outer core layer ( $H_{outer\ surface\ of\ OC}$ ), as measured in Shore C units, preferably has a lower limit of about 40 or 42 or 45 or 48 or 50 or 54 or 58 or 60 or 63 or 65 or 67 or 720 or 72 or 73 or 76 Shore C, and an upper limit of about 78 or 80 or 84 or 87 or 88 or 89 or 90 or 92 or 95 Shore C. And, the inner surface of the outer core layer ( $H_{inner\ surface\ of\ OC}$ ) or midpoint hardness of the outer core layer ( $H_{midpoint\ of\ OC}$ ), preferably has a hardness of about 40 Shore D or greater, and more preferably within a range having a lower limit of about 40 or 42 or 44 or 46 or 48 or 50 or 52 and an upper limit of about 54 or 56 or 58 or 60 or 62 or 64 or 70 or 74 or 78 or 80 or 82 or 85 or 87 or 88 or 90 Shore D. The inner surface hardness ( $H_{inner\ surface\ of\ OC}$ ) or midpoint hardness ( $H_{midpoint\ of\ OC}$ ) of the outer core layer, as measured in Shore C units, preferably has a lower limit of about 40 or 42 or 44 or 45 or 47 or 50 or 52 or 54 or 55 or 58 or 60 or 63 or 65 or 67 or 70 or 73 or 75 Shore C, and an upper limit of about 78 or 80 or 85 or 88 or 89 or 90 or 92 or 95 Shore C.

In one embodiment, the outer surface hardness of the outer core layer ( $H_{outer\ surface\ of\ OC}$ ), is less than the outer surface hardness ( $H_{inner\ core\ surface}$ ) or midpoint hardness ( $H_{midpoint\ of\ OC}$ ), of the inner core by at least 3 Shore C units and more preferably by at least 5 Shore C.

In a second embodiment, the outer surface hardness of the outer core layer ( $H_{outer\ surface\ of\ OC}$ ), is greater than the outer surface hardness ( $H_{inner\ core\ surface}$ ) or midpoint hardness ( $H_{midpoint\ of\ OC}$ ), of the inner core by at least 3 Shore C units and more preferably by at least 5 Shore C.

The core structure also has a hardness gradient across the entire core assembly. In one embodiment, the ( $H_{inner\ core\ center}$ ) is in the range of about 10 to about 60 Shore C, preferably about 13 to about 55 Shore C and more preferably about 15 to about 50 Shore C; and the ( $H_{outer\ surface\ of\ OC}$ ) is in the range of about 65 to about 96 Shore C, preferably about 68 to about 94 Shore C and more preferably about 75 to about 92 Shore C, to provide a positive hardness gradient across the core assembly.

In another embodiment, the  $H_{inner\ core\ center}$  is in the range of about 20 to about 70 Shore A and the  $H_{outer\ surface\ of\ OC}$  is in the range of about 25 to about 58 Shore D to provide a positive hardness gradient across the core assembly. The 5 gradient will vary based on several factors including, but not limited to, the dimensions of the inner core and outer core layers.

The inner core preferably has a diameter in the range of about 0.100 to about 1.100 inches. For example, the inner core may have a diameter within a range of about 0.100 to 10 about 0.500 inches. In another example, the inner core may have a diameter within a range of about 0.300 to about 0.800 inches. More particularly, the inner core may have a diameter size with a lower limit of about 0.10 or 0.12 or 0.15 or 15 0.25 or 0.30 or 0.35 or 0.45 or 0.55 inches and an upper limit of about 0.60 or 0.65 or 0.70 or 0.80 or 0.90 or 1.00 or 1.10 inches. As far as the outer core layer is concerned, it 20 preferably has a thickness in the range of about 0.100 to about 0.750 inches. For example, the lower limit of thickness may be about 0.050 or 0.100 or 0.150 or 0.200 or 0.250 or 0.300 or 0.340 or 0.400 and the upper limit may be about 0.500 or 0.550 or 0.600 or 0.650 or 0.700 or 0.750 inches.

#### Inner Core Composition

In general, foam compositions are made by forming gas 25 bubbles in a polymer mixture using a foaming (blowing) agent. As the bubbles form, the mixture expands and forms a foam composition that can be molded into an end-use product having either an open or closed cellular structure. Flexible foams generally have an open cell structure, where 30 the cells walls are incomplete and contain small holes through which liquid and air can permeate. Such flexible foams are used traditionally for automobile seats, cushioning, mattresses, and the like. Rigid foams generally have a closed cell structure, where the cell walls are continuous and 35 complete, and are used for used traditionally for automobile panels and parts, building insulation and the like. Many foams contain both open and closed cells. It also is possible to formulate flexible foams having a closed cell structure and likewise to formulate rigid foams having an open cell 40 structure.

In the present invention, the inner core (center) comprises a lightweight foam thermoplastic or thermoset polymer composition. The foam may have an open or closed cellular structure or combinations thereof and the foam structure 45 may range from a relatively rigid foam to a very flexible foam. As shown in FIG. 1, a foamed inner core (4) having a geometric center (6) and outer skin (8) may be prepared in accordance with this invention.

A wide variety of thermoplastic and thermoset materials 50 may be used in forming the foam composition of this invention including, for example, polyurethanes; polyureas; copolymers, blends and hybrids of polyurethane and polyurea; olefin-based copolymer ionomer resins (for example, Surlyn® ionomer resins and DuPont HPF® 1000 and HPF® 2000, commercially available from DuPont; Iotek® ionomers, commercially available from ExxonMobil Chemical Company; Amplify® IO ionomers of ethylene acrylic acid copolymers, commercially available from Dow Chemical Company; and Clarix® ionomer resins, commercially available from A. Schulman Inc.); polyethylene, including, for 55 example, low density polyethylene, linear low density polyethylene, and high density polyethylene; polypropylene; rubber-toughened olefin polymers; acid copolymers, for example, poly(meth)acrylic acid, which do not become part 60 of an ionomeric copolymer; plastomers; flexomers; styrene/butadiene/styrene block copolymers; styrene/ethylene-butylene/styrene block copolymers; dynamically vulcanized 65

elastomers; copolymers of ethylene and vinyl acetates; copolymers of ethylene and methyl acrylates; polyvinyl chloride resins; polyamides, poly(amide-ester) elastomers, and graft copolymers of ionomer and polyamide including, for example, Pebax® thermoplastic polyether block amides, commercially available from Arkema Inc; cross-linked trans-polyisoprene and blends thereof; polyester-based thermoplastic elastomers, such as Hytrel®, commercially available from DuPont or RiteFlex®, commercially available from Ticona Engineering Polymers; polyurethane-based thermoplastic elastomers, such as Elastollan®, commercially available from BASF; synthetic or natural vulcanized rubber; and combinations thereof. Castable polyurethanes, polyureas, and hybrids of polyurethanes-polyureas are particularly desirable because these materials can be used to make a golf ball having good playing performance properties as discussed further below. By the term, "hybrids of polyurethane and polyurea," it is meant to include copolymers and blends thereof.

Basically, polyurethane compositions contain urethane linkages formed by the reaction of a multi-functional isocyanate containing two or more NCO groups with a polyol having two or more hydroxyl groups (OH—OH) sometimes in the presence of a catalyst and other additives. Generally, polyurethanes can be produced in a single-step reaction (one-shot) or in a two-step reaction via a prepolymer or quasi-prepolymer. In the one-shot method, all of the components are combined at once, that is, all of the raw ingredients are added to a reaction vessel, and the reaction is allowed to take place. In the prepolymer method, an excess of polyisocyanate is first reacted with some amount of a polyol to form the prepolymer which contains reactive NCO groups. This prepolymer is then reacted again with a chain extender or curing agent polyol to form the final polyurethane. Polyurea compositions, which are distinct from the above-described polyurethanes, also can be formed. In general, polyurea compositions contain urea linkages formed by reacting an isocyanate group (—N=C=O) with an amine group (NH or NH<sub>2</sub>). Polyureas can be produced in similar fashion to polyurethanes by either a one shot or prepolymer method. In forming a polyurea polymer, the polyol would be substituted with a suitable polyamine. Hybrid compositions containing urethane and urea linkages also may be produced. For example, when polyurethane prepolymer is reacted with amine-terminated curing agents during the chain-extending step, any excess isocyanate groups in the prepolymer will react with the amine groups in the curing agent. The resulting polyurethane-urea composition contains urethane and urea linkages and may be referred to as a hybrid. In another example, a hybrid composition may be produced when a polyurea prepolymer is reacted with a hydroxyl-terminated curing agent. A wide variety of isocyanates, polyols, polyamines, and curing agents can be used to form the polyurethane and polyurea compositions as discussed further below.

To prepare the foamed polyurethane, polyurea, or other polymer composition, a foaming agent is introduced into the polymer formulation. In general, there are two types of foaming agents: physical foaming agents and chemical foaming agents.

#### Physical Foaming Agents.

These foaming agents typically are gasses that are introduced under high pressure directly into the polymer composition. Chlorofluorocarbons (CFCs) and partially halogenated chlorofluorocarbons are effective, but these compounds are banned in many countries because of their environmental side effects. Alternatively, aliphatic and

cyclic hydrocarbon gasses such as isobutene and pentane may be used. Inert gasses, such as carbon dioxide and nitrogen, also are suitable. With physical foaming agents, the isocyanate and polyol compounds react to form polyurethane linkages and the reaction generates heat. Foam cells are generated and as the foaming agent vaporizes, the gas becomes trapped in the cells of the foam.

#### Chemical Foaming Agents.

These foaming agents typically are in the form of powder, 10 pellets, or liquids and they are added to the composition, where they decompose or react during heating and generate gaseous by-products (for example, nitrogen or carbon dioxide). The gas is dispersed and trapped throughout the composition and foams it. For example, water may be used as the 15 foaming agent. Air bubbles are introduced into the mixture of the isocyanate and polyol compounds and water by high-speed mixing equipment. As discussed in more detail further below, the isocyanates react with the water to generate carbon dioxide which fills and expands the cells 20 created during the mixing process.

Preferably, a chemical foaming agent is used to prepare the foam compositions of this invention. Chemical blowing agents may be inorganic, such as ammonium carbonate and carbonates of alkalai metals, or may be organic, such as azo 25 and diazo compounds, such as nitrogen-based azo compounds. Suitable azo compounds include, but are not limited to, 2,2'-azobis(2-cyanobutane), 2,2'-azobis(methylbutyronitrile), azodicarbonamide, p,p'-oxybis(benzene sulfonyl hydrazide), p-toluene sulfonyl semicarbazide, p-toluene sulfonyl hydrazide. Other foaming agents include any of the 30 Celogens® sold by Crompton Chemical Corporation, and nitroso compounds, sulfonylhydrazides, azides of organic acids and their analogs, triazines, tri- and tetrazole derivatives, sulfonyl semicarbazides, urea derivatives, guanidine derivatives, and esters such as alkoxyboroxines. Also, foaming agents that liberate gasses as a result of chemical 35 interaction between components such as mixtures of acids and metals, mixtures of organic acids and inorganic carbonates, mixtures of nitriles and ammonium salts, and the hydrolytic decomposition of urea may be used. Water is a 40 preferred foaming agent. When added to the polyurethane formulation, water will react with the isocyanate groups and form carbamic acid intermediates. The carbamic acids readily decarboxylate to form an amine and carbon dioxide. The 45 newly formed amine can then further react with other isocyanate groups to form urea linkages and the carbon dioxide forms the bubbles to produce the foam.

During the decomposition reaction of certain chemical foaming agents, more heat and energy is released than is 50 needed for the reaction. Once the decomposition has started, it continues for a relatively long time period. If these foaming agents are used, longer cooling periods are generally required. Hydrazide and azo-based compounds often are used as exothermic foaming agents. On the other hand, 55 endothermic foaming agents need energy for decomposition. Thus, the release of the gasses quickly stops after the supply of heat to the composition has been terminated. If the composition is produced using these foaming agents, shorter cooling periods are needed. Bicarbonate and citric acid-based foaming agents can be used as exothermic foaming agents.

Other suitable foaming agents include expandable gas-containing microspheres. Exemplary microspheres consist of an acrylonitrile polymer shell encapsulating a volatile 60 gas, such as isopentane gas. This gas is contained within the sphere as a blowing agent. In their unexpanded state, the diameter of these hollow spheres range from 10 to 17  $\mu\text{m}$

and have a true density of 1000 to 1300 kg/m<sup>3</sup>. When heated, the gas inside the shell increases its pressure and the thermoplastic shell softens, resulting in a dramatic increase of the volume of the microspheres. Fully expanded, the volume of the microspheres will increase more than 40 times (typical diameter values would be an increase from 10 to 40 µm), resulting in a true density below 30 kg/m<sup>3</sup> (0.25 lbs/gallon). Typical expansion temperatures range from 80-190° C. (176-374° F.). Such expandable microspheres are commercially available as Expance® from Expance of Sweden or Akzo Nobel.

As an alternative to chemical and physical foaming agents or in addition to such foaming agents, as described above, other types of fillers that lower the specific gravity of the composition can be used in accordance with this invention. For example, polymeric, ceramic, and glass unfilled microspheres having a density of 0.1 to 1.0 g/cc and an average particle size of 10 to 250 microns can be used to help lower specific gravity of the composition and achieve the desired density and physical properties.

Additionally, BASF polyurethane materials sold under the trade name Cellasto® and Elastocell®, microcellular polyurethanes, Elastopor® H that is a closed-cell polyurethane rigid foam, Elastoflex® W flexible foam systems, Elastoflex® E semiflexible foam systems, Elastofoam® flexible integrally-skinning systems, Elastolit® D/K/R integral rigid foams, Elastopan® S, Elastollan® thermoplastic polyurethane elastomers (TPUs), and the like may be used in accordance with the present invention. Furthermore, BASF closed-cell, pre-expanded thermoplastic (TPU) polyurethane foam, available under the mark, Infinergy™ also may be used to form the foam centers of the golf balls in accordance with this invention. It also is believed these foam materials would be useful in forming non-center foamed layers in a variety of golf ball constructions. Such closed-cell, pre-expanded TPU foams are described in Prissok et al., US Patent Applications 2012/0329892; 2012/0297513; and 2013/0227861; and U.S. Pat. No. 8,282,851 the disclosures of which are hereby incorporated by reference. Bayer also produces a variety of materials sold as Texin® TPUs, Baytec® and Vulkollan® elastomers, Baymer® rigid foams, Baydur® integral skinning foams, Bayfit® flexible foams available as castable, RIM grades, sprayable, and the like that may be used. Additional foam materials that may be used herein include polyisocyanurate foams and a variety of "thermoplastic" foams, which may be cross-linked to varying extents using free-radical (for example, peroxide) or radiation cross-linking (for example, UV, IR, Gamma, EB irradiation). Also, foams may be prepared from polybutadiene, polystyrene, polyolefin (including metallocene and other single site catalyzed polymers), ethylene vinyl acetate (EVA), acrylate copolymers, such as EMA, EBA, Nucrel®-type acid co and terpolymers, ethylene propylene rubber (such as EPR, EPDM, and any ethylene copolymers), styrene-butadiene, and SEBS (any Kraton-type), PVC, PVDC, CPE (chlorinated polyethylene). Epoxy foams, urea-formaldehyde foams, latex foams and sponge, silicone foams, fluoropolymer foams and syntactic foams (hollow sphere filled) also may be used. In particular, silicone foams may be used. For example, the inner core (center) may be made of a silicone foam rubber and the surrounding outer core layer may be made of a non-foamed thermoset or thermoplastic composition. The silicone foam rubber composition has good thermal stability. Thus, the thermoset or thermoplastic composition may be molded more effectively over the inner core, and the chemical and physical properties of the inner core will not degrade substantially.

In addition to the polymer and foaming agent, the foam composition also may include other ingredients such as, for example, fillers, cross-linking agents, chain extenders, surfactants, dyes and pigments, coloring agents, fluorescent agents, adsorbents, stabilizers, softening agents, impact modifiers, antioxidants, antiozonants, and the like. The formulations used to prepare the polyurethane foam compositions of this invention preferably contain a polyol, polyisocyanate, water, an amine or hydroxyl curing agent, surfactant, and a catalyst as described further below.

#### Fillers.

The polyurethane foam composition may contain fillers such as, for example, mineral filler particulate. Suitable mineral filler particulates include compounds such as zinc oxide, limestone, silica, mica, barytes, lithopone, zinc sulfide, talc, calcium carbonate, magnesium carbonate, clays, powdered metals and alloys such as bismuth, brass, bronze, cobalt, copper, iron, nickel, tungsten, aluminum, tin, precipitated hydrated silica, fumed silica, mica, calcium metasilicate, barium sulfate, zinc sulfide, lithopone, silicates, silicon carbide, diatomaceous earth, carbonates such as calcium or magnesium or barium carbonate, sulfates such as calcium or magnesium or barium sulfate. Adding fillers to the foam composition provides many benefits including helping improve the stiffness and strength of the composition. The mineral fillers tend to help decrease the size of the foam cells and increase cell density. The mineral fillers also tend to help improve the physical properties of the foam such as hardness, compression set, and tensile strength. However, in the present invention, it is important the concentration of fillers in the foam composition be not so high as to substantially increase the specific gravity (density) of the composition. Particularly, the specific gravity of the inner core is maintained such that is less than the specific gravity of the outer core layer as discussed further below. The foam composition may contain some fillers; provided however, the specific gravity of the foam composition (inner core) is kept less than the composition of the surrounding outer core layer. In one embodiment, the foam composition is substantially free of fillers. In another embodiment, the foam composition contains no fillers and consists of a mixture of polyisocyanate, polyol, and curing agent, surfactant, catalyst, and water, the water being added in sufficient amount to cause the mixture to foam as discussed above.

If filler is added to the foam composition, clay particulate fillers are particularly suitable. The clay particulate fillers include Garamite® mixed mineral thixotropes and Cloisite® and Nanofil® nanoclays, commercially available from Southern Clay Products, Inc., and Nanomax® and Nanomer® nanoclays, commercially available from Nanocor, Inc may be used. Other nano-scale materials such as nanotubes and nanoflakes also may be used. Also, talc particulate (e.g., Luzenac HAR® high aspect ratio talcs, commercially available from Luzenac America, Inc.), glass (e.g., glass flake, milled glass, and microglass), and combinations thereof may be used. Metal oxide fillers have good heat-stability and may be added including, for example, aluminum oxide, zinc oxide, tin oxide, barium sulfate, zinc sulfate, calcium oxide, calcium carbonate, zinc carbonate, barium carbonate, tungsten, tungsten carbide, and lead silicate fillers. Other metal fillers such as, for example, particulate; powders; flakes; and fibers of copper, steel, brass, tungsten, titanium, aluminum, magnesium, molybdenum, cobalt, nickel, iron, lead, tin, zinc, barium, bismuth, bronze, silver, gold, and platinum, and alloys and combinations thereof also may be added to the foam composition.

## Surfactants.

The foam composition also may contain surfactants to stabilize the foam and help control the foam cell size and structure. In one preferred version, the foam composition includes silicone surfactant. In general, the silicone surfactant helps regulate the foam cell size and stabilizes the cell walls to prevent the cells from collapsing. As discussed above, the liquid reactants react to form the foam rapidly. The "liquid" foam develops into solid silicone foam in a relatively short period of time. If a silicone surfactant is not added, the gas-liquid interface between the liquid reactants and expanding gas bubbles may not support the stress. As a result, the cell window can crack or rupture and there can be cell wall drainage. In turn, the foam can collapse on itself. Adding a silicone surfactant helps create a surface tension gradient along the gas-liquid interface and helps reduce cell wall drainage. The silicone surfactant has a relatively low surface tension and thus can lower the surface tension of the foam. It is believed the silicone surfactant orients itself the foam cell walls and lowers the surface tension to create the surface tension gradient. Blowing efficiency and nucleation are supported by adding the silicone surfactant and thus more bubbles are created in the system. The silicone surfactant also helps create a greater number of smaller sized foam cells and increases the closed cell content of the foam due to the surfactant's lower surface tension. Thus, the cell structure in the foam is maintained as the gas is prevented from diffusing out through the cell walls. Along with the decrease in cell size, there is a decrease in thermal conductivity. The resulting foam material also tends to have greater compression strength and modulus. These improved physical properties may be due to the increase in closed cell content and smaller cell size.

As discussed further below, in one preferred embodiment, the specific gravity (density) of the foam inner core is less than the specific gravity of the outer core. If mineral filler or other additives are included in the foam composition, they should not be added in an amount that would increase the specific gravity (density) of the foam inner core to a level such that it would be greater than the specific gravity of the outer core layer. If the ball's mass is concentrated towards the outer surface (for example, outer core layers), and the outer core layer has a higher specific gravity than the inner core, the ball has a relatively high Moment of Inertia (MOI). In such balls, most of the mass is located away from the ball's axis of rotation and thus more force is needed to generate spin. These balls have a generally low spin rate as the ball leaves the club's face after contact between the ball and club. Such core structures (wherein the specific gravity of the outer core is greater than the specific gravity of the inner core) is preferred in the present invention. Thus, in one preferred embodiment, the concentration of mineral filler particulate in the foam composition is in the range of about 0.1 to about 9.0% by weight.

## Properties of Polyurethane Foams

The polyurethane foam compositions of this invention have numerous chemical and physical properties making them suitable for core assemblies in golf balls. For example, there are properties relating to the reaction of the isocyanate and polyol components and blowing agent, particularly "cream time," "gel time," "rise time," "tack-free time," and "free-rise density." In general, cream time refers to the time period from the point of mixing the raw ingredients together to the point where the mixture turns cloudy in appearance or changes color and begins to rise from its initial stable state. Normally, the cream time of the foam compositions of this invention is within the range of about 20 to about 240

seconds. In general, gel time refers to the time period from the point of mixing the raw ingredients together to the point where the expanded foam starts polymerizing/gelling. Rise time generally refers to the time period from the point of mixing the raw ingredients together to the point where the reacted foam has reached its largest volume or maximum height. The rise time of the foam compositions of this invention typically is in the range of about 60 to about 360 seconds. Tack-free time generally refers to the time it takes for the reacted foam to lose its tackiness, and the foam compositions of this invention normally have a tack-free time of about 60 to about 3600 seconds. Free-rise density refers to the density of the resulting foam when it is allowed to rise unrestricted without a cover or top being placed on the mold.

The density of the foam is an important property and is defined as the weight per unit volume (typically, g/cm<sup>3</sup>) and can be measured per ASTM D-1622. The hardness, stiffness, and load-bearing capacity of the foam are independent of the foam's density, although foams having a high density typically have high hardness and stiffness. Normally, foams having higher densities have higher compression strength. Surprisingly, the foam compositions used to produce the inner core of the golf balls per this invention have a relatively low density; however, the foams are not necessarily soft and flexible, rather, they may be relatively firm, rigid, or semi-rigid depending upon the desired golf ball properties. Tensile strength, tear-resistance, and elongation generally refer to the foam's ability to resist breaking or tearing, and these properties can be measured per ASTM D-1623. The durability of foams is important, because introducing fillers and other additives into the foam composition can increase the tendency of the foam to break or tear apart. In general, the tensile strength of the foam compositions of this invention is in the range of about 20 to about 1000 psi (parallel to the foam rise) and about 50 to about 1000 psi (perpendicular to the foam rise) as measured per ASTM D-1623 at 23° C. and 50% relative humidity (RH). Meanwhile, the flex modulus of the foams of this invention is generally in the range of about 5 to about 45 kPa as measured per ASTM D-790, and the foams generally have a compressive modulus of 200 to 50,000 psi.

In another test, compression strength is measured on an Instron machine according to ASTM D-1621. The foam is cut into blocks and the compression strength is measured as the force required for compressing the block by 10%. In general, the compressive strength of the foam compositions of this invention is in the range of about 100 to about 1800 psi (parallel and perpendicular to the foam rise) as measured per ASTM D-1621 at 23° C. and 50% relative humidity (RH). The test is conducted perpendicular to the rise of the foam or parallel to the rise of the foam. The Percentage (%) of Compression Set also can be used. This is a measure of the permanent deformation of a foam sample after it has been compressed between two metal plates under controlled time and temperature condition (standard—22 hours at 70° C. (158° F.)). The foam is compressed to a thickness given as a percentage of its original thickness that remained "set." Preferably, the Compression Set of the foam is less than ten percent (10%), that is, the foam recovers to a point of 90% or greater of its original thickness.

The foam compositions of this invention may be prepared using different methods. In one preferred embodiment, the method involves preparing a castable composition comprising a reactive mixture of a polyisocyanate, polyol, water, curing agent, surfactant, and catalyst. A motorized mixer can be used to mix the starting ingredients together and form a

reactive liquid mixture. Alternatively, the ingredients can be manually mixed together. An exothermic reaction occurs when the ingredients are mixed together and this continues as the reactive mixture is dispensed into the mold cavities (otherwise referred to as half-molds or mold cups).

#### Outer Core Composition

As discussed above, a two-layered or dual-core is preferably made, wherein the inner core (center) is surrounded by an outer core layer, and the center is made from a foamed composition. In one preferred embodiment, the outer core layer is made from a non-foamed thermoset composition and more preferably from a non-foamed thermoset rubber composition.

Suitable thermoset rubber materials that may be used to form the outer core layer include, but are not limited to, polybutadiene, polyisoprene, ethylene propylene rubber ("EPR"), ethylene-propylene-diene ("EPDM") rubber, styrene-butadiene rubber, styrenic block copolymer rubbers (such as "SI", "SIS", "SB", "SBS", "SIBS", and the like, where "S" is styrene, "I" is isobutylene, and "B" is butadiene), polyalkenamers such as, for example, polyoctenamer, butyl rubber, halobutyl rubber, polystyrene elastomers, polyethylene elastomers, polyurethane elastomers, polyurea elastomers, metallocene-catalyzed elastomers and plasto-  
mers, copolymers of isobutylene and p-alkylstyrene, halogenated copolymers of isobutylene and p-alkylstyrene, copolymers of butadiene with acrylonitrile, polychloroprene, alkyl acrylate rubber, chlorinated isoprene rubber, acrylonitrile chlorinated isoprene rubber, and blends of two or more thereof. Preferably, the outer core layer is formed from a polybutadiene rubber composition.

The thermoset rubber composition may be cured using conventional curing processes. Suitable curing processes include, for example, peroxide-curing, sulfur-curing, high-energy radiation, and combinations thereof. Preferably, the rubber composition contains a free-radical initiator selected from organic peroxides, high energy radiation sources capable of generating free-radicals, and combinations thereof. In one preferred version, the rubber composition is peroxide-cured. Suitable organic peroxides include, but are not limited to, dicumyl peroxide; n-butyl-4,4-di(t-butylperoxy) valerate; 1,1-di(t-butylperoxy)3,3,5-trimethylcyclohexane; 2,5-dimethyl-2,5-di(t-butylperoxy) hexane; di-t-butyl peroxide; di-t-amyl peroxide; t-butyl peroxide; t-butyl cumyl peroxide; 2,5-dimethyl-2,5-di(t-butylperoxy)hexyne-3; di(2-t-butyl-peroxyisopropyl)benzene; dilaurol peroxide; dibenzoyl peroxide; t-butyl hydroperoxide; and combinations thereof. In a particular embodiment, the free radical initiator is dicumyl peroxide, including, but not limited to Perkadox® BC, commercially available from Akzo Nobel. Peroxide free-radical initiators are generally present in the rubber composition in an amount of at least 0.05 parts by weight per 100 parts of the total rubber, or an amount within the range having a lower limit of 0.05 parts or 0.1 parts or 1 part or 1.25 parts or 1.5 parts or 2.5 parts or 5 parts by weight per 100 parts of the total rubbers, and an upper limit of 2.5 parts or 3 parts or 5 parts or 6 parts or 10 parts or 15 parts by weight per 100 parts of the total rubber. Concentrations are in parts per hundred (phr) unless otherwise indicated. As used herein, the term, "parts per hundred," also known as "phr" or "pph" is defined as the number of parts by weight of a particular component present in a mixture, relative to 100 parts by weight of the polymer component. Mathematically, this can be expressed as the weight of an ingredient divided by the total weight of the polymer, multiplied by a factor of 100.

The rubber compositions may further include a reactive cross-linking co-agent. Suitable co-agents include, but are not limited to, metal salts of unsaturated carboxylic acids having from 3 to 8 carbon atoms; unsaturated vinyl compounds and polyfunctional monomers (e.g., trimethylolpropane trimethacrylate); phenylene bismaleimide; and combinations thereof. Particular examples of suitable metal salts include, but are not limited to, one or more metal salts of acrylates, diacrylates, methacrylates, and dimethacrylates, 5 wherein the metal is selected from magnesium, calcium, zinc, aluminum, lithium, and nickel. In a particular embodiment, the co-agent is selected from zinc salts of acrylates, diacrylates, methacrylates, and dimethacrylates. In another particular embodiment, the agent is zinc diacrylate (ZDA). 10 When the co-agent is zinc diacrylate and/or zinc dimethacrylate, the co-agent is typically included in the rubber composition in an amount within the range having a lower limit of 1 or 5 or 10 or 15 or 19 or 20 parts by weight per 100 parts of the total rubber, and an upper limit of 24 or 25 15 or 30 or 35 or 40 or 45 or 50 or 60 parts by weight per 100 parts of the base rubber.

Radical scavengers such as a halogenated organosulfur, 20 organic disulfide, or inorganic disulfide compounds may be added to the rubber composition. These compounds also 25 may function as "soft and fast agents." As used herein, "soft and fast agent" means any compound or a blend thereof that is capable of making a core: 1) softer (having a lower compression) at a constant "coefficient of restitution" (COR); and/or 2) faster (having a higher COR at equal 30 compression), when compared to a core equivalently prepared without a soft and fast agent. Preferred halogenated organosulfur compounds include, but are not limited to, pentachlorothiophenol (PCTP) and salts of PCTP such as zinc pentachlorothiophenol (ZnPCTP). Using PCTP and 35 ZnPCTP in golf ball inner cores helps produce softer and faster inner cores. The PCTP and ZnPCTP compounds help increase the resiliency and the coefficient of restitution of the core. In a particular embodiment, the soft and fast agent is selected from ZnPCTP, PCTP, ditolyl disulfide, diphenyl 40 disulfide, dixylyl disulfide, 2-nitroresorcinol, and combinations thereof.

In addition, the rubber compositions may include antioxidants. Also, processing aids such as high molecular weight 45 organic acids and salts thereof may be added to the composition. Other ingredients such as accelerators, dyes and pigments, wetting agents, surfactants, plasticizers, coloring agents, fluorescent agents, stabilizers, softening agents, impact modifiers, antiozonants, as well as other additives known in the art may be added to the rubber composition. The rubber composition also may include filler(s) such as 50 materials selected from carbon black, clay and nanoclay particles as discussed above, talc (e.g., Luzenac HAR® high aspect ratio talcs, commercially available from Luzenac America, Inc.), glass (e.g., glass flake, milled glass, and microglass), mica and mica-based pigments (e.g., Iridin® pearl luster pigments, commercially available from The Merck Group), and combinations thereof. Metal fillers such as, for example, particulate; powders; flakes; and fibers of 55 copper, steel, brass, tungsten, titanium, aluminum, magnesium, molybdenum, cobalt, nickel, iron, lead, tin, zinc, barium, bismuth, bronze, silver, gold, and platinum, and alloys and combinations thereof also may be added to the rubber composition to adjust the specific gravity of the composition as needed. As discussed above, the inner core 60 layer preferably has a specific gravity (density) less than the outer core layer's specific gravity. Thus, metal or other fillers may be added to the polybutadiene rubber composition (or

other thermoset material) used to form the outer core layer, and the specific gravity of the outer core remains greater than the specific gravity of the inner core.

Examples of commercially-available polybutadiene rubbers that can be used in accordance with this invention, include, but are not limited to, BR 01 and BR 1220, available from BST Elastomers of Bangkok, Thailand; SE BR 1220LA and SE BR1203, available from DOW Chemical Co of Midland, Mich.; BUDENE 1207, 1207s, 1208, and 1280 available from Goodyear, Inc of Akron, Ohio; BR 01, 51 and 730, available from Japan Synthetic Rubber (JSR) of Tokyo, Japan; BUNA CB 21, CB 22, CB 23, CB 24, CB 25, CB 29 MES, CB 60, CB Nd 60, CB 55 NF, CB 70 B, CB KA 8967, and CB 1221, available from Lanxess Corp. of Pittsburgh, Pa.; BR1208, available from LG Chemical of Seoul, South Korea; UBEPOL BR130B, BR150, BR150B, BR150L, BR230, BR360L, BR710, and VCR617, available from UBE Industries, Ltd. of Tokyo, Japan; EUROPRENE NEO-CIS BR 60, INTENE 60 AF and P30AF, and EUROPRENE BR HV80, available from Polimeri Europa of Rome, Italy; AFDENE 50 and NEODENE BR40, BR45, BR50 and BR60, available from Karbochem (PTY) Ltd. of Bruma, South Africa; KBR 01, NdBr 40, NdBr-45, NdBr 60, KBR 710S, KBR 710H, and KBR 750, available from Kumho Petrochemical Co., Ltd. Of Seoul, South Korea; DIENE 55NF, 70AC, and 320 AC, available from Firestone Polymers of Akron, Ohio; and PBR-Nd Group II and Group III, available from Nizhnekamskneftekhim, Inc. of Nizhnekamsk, Tartarstan Republic.

The polybutadiene rubber is used in an amount of at least about 5% by weight based on total weight of composition and is generally present in an amount of about 5% to about 100%, or an amount within a range having a lower limit of 5% or 10% or 20% or 30% or 40% or 50% and an upper limit of 55% or 60% or 70% or 80% or 90% or 95% or 100%. Preferably, the concentration of polybutadiene rubber is about 40 to about 95 weight percent. If desirable, lesser amounts of other thermoset materials may be incorporated into the base rubber. Such materials include the rubbers discussed above, for example, cis-polyisoprene, trans-polyisoprene, balata, polychloroprene, polynorbornene, poly-octenamer, polypentenamer, butyl rubber, EPR, EPDM, styrene-butadiene, and the like.

As discussed above, in one preferred embodiment, a thermoset rubber composition is used to form the outer core. In alternative embodiments, the outer core layer is made from a thermoplastic material, for example, an ionomer composition.

Suitable ionomer compositions include partially-neutralized ionomers and highly-neutralized ionomers (HNPs), including ionomers formed from blends of two or more partially-neutralized ionomers, blends of two or more highly-neutralized ionomers, and blends of one or more partially-neutralized ionomers with one or more highly-neutralized ionomers. For purposes of the present disclosure, "HNP" refers to an acid copolymer after at least 70% of all acid groups present in the composition are neutralized.

Preferred ionomers are salts of O/X- and O/X/Y-type acid copolymers, wherein O is an  $\alpha$ -olefin, X is a  $C_3$ - $C_8$   $\alpha,\beta$ -ethylenically unsaturated carboxylic acid, and Y is a softening monomer. O is preferably selected from ethylene and propylene. X is preferably selected from methacrylic acid, acrylic acid, ethacrylic acid, crotonic acid, and itaconic acid. Methacrylic acid and acrylic acid are particularly preferred. Y is preferably selected from (meth)acrylate and alkyl(meth)acrylates wherein the alkyl groups have from 1 to 8 carbon

atoms, including, but not limited to, n-butyl(meth)acrylate, isobutyl(meth)acrylate, methyl(meth)acrylate, and ethyl (meth)acrylate.

Preferred O/X and O/X/Y-type copolymers include, without limitation, ethylene acid copolymers, such as ethylene/(meth)acrylic acid, ethylene/(meth)acrylic acid/maleic anhydride, ethylene/(meth)acrylic acid/maleic acid mono-ester, ethylene/maleic acid, ethylene/maleic acid mono-ester, ethylene/(meth)acrylic acid/n-butyl(meth)acrylate, ethylene/(meth)acrylic acid/iso-butyl(meth)acrylate, ethylene/(meth)acrylic acid/methyl(meth)acrylate, ethylene/(meth)acrylic acid/ethyl(meth)acrylate terpolymers, and the like. The term, "copolymer," as used herein, includes polymers having two types of monomers, those having three types of monomers, and those having more than three types of monomers. Preferred  $\alpha,\beta$ -ethylenically unsaturated mono- or dicarboxylic acids are (meth)acrylic acid, ethacrylic acid, maleic acid, crotonic acid, fumaric acid, itaconic acid. (Meth)acrylic acid is most preferred. As used herein, "(meth)acrylic acid" means methacrylic acid and/or acrylic acid. Likewise, "(meth)acrylate" means methacrylate and/or acrylate.

In a particularly preferred version, highly neutralized E/X- and E/X/Y-type acid copolymers, wherein E is ethylene, X is a  $C_3$ - $C_8$   $\alpha,\beta$ -ethylenically unsaturated carboxylic acid, and Y is a softening monomer are used. X is preferably selected from methacrylic acid, acrylic acid, ethacrylic acid, crotonic acid, and itaconic acid. Methacrylic acid and acrylic acid are particularly preferred. Y is preferably an acrylate selected from alkyl acrylates and aryl acrylates and preferably selected from (meth)acrylate and alkyl(meth)acrylates wherein the alkyl groups have from 1 to 8 carbon atoms, including, but not limited to, n-butyl(meth)acrylate, isobutyl (meth)acrylate, methyl(meth)acrylate, and ethyl(meth)acrylate. Preferred E/X/Y-type copolymers are those wherein X is (meth)acrylic acid and/or Y is selected from (meth) acrylate, n-butyl(meth)acrylate, isobutyl(meth)acrylate, methyl(meth)acrylate, and ethyl(meth)acrylate. More preferred E/X/Y-type copolymers are ethylene/(meth)acrylic acid/n-butyl acrylate, ethylene/(meth)acrylic acid/methyl acrylate, and ethylene/(meth)acrylic acid/ethyl acrylate.

The amount of ethylene in the acid copolymer is typically at least 15 wt. %, preferably at least 25 wt. %, more preferably least 40 wt. %, and even more preferably at least 60 wt. %, based on total weight of the copolymer. The amount of  $C_3$  to  $C_8$   $\alpha,\beta$ -ethylenically unsaturated mono- or dicarboxylic acid in the acid copolymer is typically from 1 wt. % to 35 wt. %, preferably from 5 wt. % to 30 wt. %, more preferably from 5 wt. % to 25 wt. %, and even more preferably from 10 wt. % to 20 wt. %, based on total weight of the copolymer. The amount of optional softening comonomer in the acid copolymer is typically from 0 wt. % to 50 wt. %, preferably from 5 wt. % to 40 wt. %, more preferably from 10 wt. % to 35 wt. %, and even more preferably from 20 wt. % to 30 wt. %, based on total weight of the copolymer. "Low acid" and "high acid" ionomeric polymers, as well as blends of such ionomers, may be used. In general, low acid ionomers are considered to be those containing 16 wt. % or less of acid moieties, whereas high acid ionomers are considered to be those containing greater than 16 wt. % of acid moieties.

The various O/X, E/X, O/X/Y, and E/X/Y-type copolymers are at least partially neutralized with a cation source, optionally in the presence of a high molecular weight organic acid, such as those disclosed in Rajagopalan et al., U.S. Pat. No. 6,756,436, the entire disclosure of which is hereby incorporated herein by reference. The acid copoly-

mer can be reacted with the optional high molecular weight organic acid and the cation source simultaneously, or prior to the addition of the cation source. Suitable cation sources include, but are not limited to, metal ion sources, such as compounds of alkali metals, alkaline earth metals, transition metals, and rare earth elements; ammonium salts and mono-amine salts; and combinations thereof. Preferred cation sources are compounds of magnesium, sodium, potassium, cesium, calcium, barium, manganese, copper, zinc, lead, tin, aluminum, nickel, chromium, lithium, and rare earth metals. The amount of cation used in the composition is readily determined based on desired level of neutralization. As discussed above, for HNP compositions, the acid groups are neutralized to 70% or greater, preferably 70 to 100%, more preferably 90 to 100%. In one embodiment, an excess amount of neutralizing agent, that is, an amount greater than the stoichiometric amount needed to neutralize the acid groups, may be used. That is, the acid groups may be neutralized to 100% or greater, for example 110% or 120% or greater. In other embodiments, partially-neutralized compositions are prepared, wherein 10% or greater, normally 30% or greater of the acid groups are neutralized. When aluminum is used as the cation source, it is preferably used at low levels with another cation such as zinc, sodium, or lithium, since aluminum has a dramatic effect on melt flow reduction and cannot be used alone at high levels. For example, aluminum is used to neutralize about 10% of the acid groups and sodium is added to neutralize an additional 90% of the acid groups.

"Ionic plasticizers" such as organic acids or salts of organic acids, particularly fatty acids, may be added to the ionomer resin. Such ionic plasticizers are used to make conventional ionomer composition more processable as described in the above-mentioned U.S. Pat. No. 6,756,436. In the present invention such ionic plasticizers are optional. In one preferred embodiment, a thermoplastic ionomer composition is made by neutralizing about 70 wt % or more of the acid groups without the use of any ionic plasticizer. On the other hand, in some instances, it may be desirable to add a small amount of ionic plasticizer, provided that it does not adversely affect the heat-resistance properties of the composition. For example, the ionic plasticizer may be added in an amount of about 10 to about 60 weight percent (wt. %) of the composition, more preferably 30 to 55 wt. %.

The organic acids may be aliphatic, mono- or multi-functional (saturated, unsaturated, or multi-unsaturated) organic acids. Salts of these organic acids may also be employed. Suitable fatty acid salts include, for example, metal stearates, laureates, oleates, palmitates, pelargonates, and the like. For example, fatty acid salts such as zinc stearate, calcium stearate, magnesium stearate, barium stearate, and the like can be used. The salts of fatty acids are generally fatty acids neutralized with metal ions. The metal cation salts provide the cations capable of neutralizing (at varying levels) the carboxylic acid groups of the fatty acids. Examples include the sulfate, carbonate, acetate and hydroxide salts of metals such as barium, lithium, sodium, zinc, bismuth, chromium, cobalt, copper, potassium, strontium, titanium, tungsten, magnesium, cesium, iron, nickel, silver, aluminum, tin, or calcium, and blends thereof. It is preferred the organic acids and salts be relatively non-migratory (they do not bloom to the surface of the polymer under ambient temperatures) and non-volatile (they do not volatilize at temperatures required for melt-blending).

Other suitable thermoplastic polymers that may be used to form the inner cover layer include, but are not limited to, the following polymers (including homopolymers, copolymers, and derivatives thereof)

- 5 (a) polyesters, particularly those modified with a compatibilizing group such as sulfonate or phosphonate, including modified poly(ethylene terephthalate), modified poly(butylene terephthalate), modified poly(propylene terephthalate), modified poly(trimethylene terephthalate), modified poly(ethylene naphthalene), and those disclosed in U.S. Pat. Nos. 6,353,050, 6,274, 298, and 6,001,930, the entire disclosures of which are hereby incorporated herein by reference, and blends of two or more thereof;
- (b) polyamides, polyamide-ethers, and polyamide-esters, and those disclosed in U.S. Pat. Nos. 6,187,864, 6,001, 930, and 5,981,654, the entire disclosures of which are hereby incorporated herein by reference, and blends of two or more thereof;
- (c) polyurethanes, polyureas, polyurethane-polyurea hybrids, and blends of two or more thereof;
- (d) fluoropolymers, such as those disclosed in U.S. Pat. Nos. 5,691,066, 6,747,110 and 7,009,002, the entire disclosures of which are hereby incorporated herein by reference, and blends of two or more thereof;
- (e) polystyrenes, such as poly(styrene-co-maleic anhydride), acrylonitrile-butadiene-styrene, poly(styrene sulfonate), polyethylene styrene, and blends of two or more thereof;
- (f) polyvinyl chlorides and grafted polyvinyl chlorides, and blends of two or more thereof;
- (g) polycarbonates, blends of polycarbonate/acrylonitrile-butadiene-styrene, blends of polycarbonate/polyurethane, blends of polycarbonate/polyester, and blends of two or more thereof;
- (h) polyethers, such as polyarylene ethers, polyphenylene oxides, block copolymers of alkenyl aromatics with vinyl aromatics and polyamicesters, and blends of two or more thereof;
- (i) polyimides, polyetherketones, polyamideimides, and blends of two or more thereof; and
- (j) polycarbonate/polyester copolymers and blends.

It also is recognized that thermoplastic materials can be "converted" into thermoset materials by cross-linking the polymer chains so they form a network structure, and such cross-linked thermoplastic materials may be used to form the inner cover layers in accordance with this invention. For example, thermoplastic polyolefins such as linear low density polyethylene (LLDPE), low density polyethylene (LDPE), and high density polyethylene (HDPE) may be cross-linked to form bonds between the polymer chains. The cross-linked thermoplastic material typically has improved physical properties and strength over non-cross-linked thermoplastics, particularly at temperatures above the crystalline melting point. Preferably a partially or fully-neutralized ionomer, as described above, is covalently cross-linked to render it into a thermoset composition (that is, it contains at least some level of covalent, irreversible cross-links). Thermoplastic polyurethanes and polyureas also may be converted into thermoset materials in accordance with the present invention.

Modifications in the thermoplastic polymeric structure of thermoplastics can be induced by a number of methods, including exposing the thermoplastic material to high-energy radiation or through a chemical process using peroxide. Radiation sources include, but are not limited to, gammas, electrons, neutrons, protons, x-rays, helium nuclei, or

the like. Gamma radiation, typically using radioactive cobalt atoms and allows for considerable depth of treatment, if necessary. For core layers requiring lower depth of penetration, electron-beam accelerators or UV and IR light sources can be used. Useful UV and IR irradiation methods are disclosed in U.S. Pat. Nos. 6,855,070 and 7,198,576, which are incorporated herein by reference. The thermoplastic core layers may be irradiated at dosages greater than 0.05 Mrd, preferably ranging from 1 Mrd to 20 Mrd, more preferably from 2 Mrd to 15 Mrd, and most preferably from 4 Mrd to 10 Mrd. In one preferred embodiment, the cores are irradiated at a dosage from 5 Mrd to 8 Mrd and in another preferred embodiment, the cores are irradiated with a dosage from 0.05 Mrd to 3 Mrd, more preferably 0.05 Mrd to 1.5 Mrd.

The cross-linked thermoplastic material may be created by exposing the thermoplastic to: 1) a high-energy radiation treatment, such as electron beam or gamma radiation, such as disclosed in U.S. Pat. No. 5,891,973, which is incorporated by reference herein, 2) lower energy radiation, such as ultra-violet (UV) or infra-red (IR) radiation; 3) a solution treatment, such as an isocyanate or a silane; 4) incorporation of additional free radical initiator groups in the thermoplastic prior to molding; and/or 5) chemical modification, such as esterification or saponification, to name a few.

#### Core Structure—Specific Gravity (Density)

As discussed above, the core of the golf ball of this invention preferably has a dual-layered structure comprising inner (center) and outer core layers. The specific gravity (density) of the respective core layers is an important property, because they affect the Moment of Inertia (MOI) of the ball. In one preferred embodiment, the inner core layer has a relatively low specific gravity ("SG<sub>inner</sub>"). For example, the inner core layer may have a specific gravity within a range having a lower limit of about 0.20 or 0.34 or 0.28 or 0.30 or 0.34 or 0.35 or 0.40 or 0.42 or 0.44 or 0.50 or 0.53 or 0.57 or 0.60 or 0.62 or 0.65 or 0.70 or 0.75 or 0.77 or 0.80 g/cc and an upper limit of about 0.82 or 0.85 or 0.88 or 0.90 or 0.95 or 1.00 or 1.10 or 1.15 or 1.18 or 1.25 g/cc. In a particularly preferred version, the inner core has a specific gravity of about 0.50 g/cc. Also, as discussed below, the specific gravity of the inner core may vary at different particular points of the inner core structure. That is, there may be a specific gravity gradient in the inner core. For example, in one preferred version, the geometric center of the inner core has a density in the range of about 0.25 to about 0.75 g/cc; while the outer skin of the inner core has a density in the range of about 0.75 to about 1.35 g/cc. By the term, "specific gravity of the inner core layer" ("SG<sub>inner</sub>"), it is generally meant the specific gravity of the outer core layer as measured at any point in the outer core layer.

Meanwhile, the outer core layer preferably has a relatively high specific gravity (SG<sub>outer</sub>). Thus, the specific gravity of the inner core layer (SG<sub>inner</sub>) is preferably less than the specific gravity of the outer core layer (SG<sub>outer</sub>). By the term, "specific gravity of the outer core layer" ("SG<sub>outer</sub>"), it is generally meant the specific gravity of the outer core layer as measured at any point in the outer core layer. The specific gravity values at different particular points in the outer core layer may vary. That is, there may be specific gravity gradients in the outer core layer similar to the gradients found in the inner core. For example, the outer core layer may have a specific gravity within a range having a lower limit of about 0.60 or 0.64 or 0.66 or 0.70 or 0.72 or 0.75 or 0.78 or 0.80 or 0.82 or 0.85 or 0.88 or 0.90 g/cc and an upper limit of about 0.95 or 1.00 or 1.05 or 1.10 or 1.14 or 1.20 or 1.25 or 1.30 or 1.36 or 1.40 or 1.42 or 1.48 or 1.50 or 1.60

or 1.66 or 1.70 or 1.75 or 2.00 g/cc. In a particularly preferred version, the inner core has a specific gravity of about 1.05 g/cc.

In general, the specific gravities of the respective pieces of an object affect the Moment of Inertia (MOI) of the object. The Moment of Inertia of a ball (or other object) about a given axis generally refers to how difficult it is to change the ball's angular motion about that axis. If the ball's mass is concentrated towards the center, less force is required to change its rotational rate, and the ball has a relatively low Moment of Inertia. In such balls, the center piece (that is, the inner core) has a higher specific gravity than the outer piece (that is, the outer core layer). In such balls, most of the mass is located close to the ball's axis of rotation and less force is needed to generate spin. Thus, the ball has a generally high spin rate as the ball leaves the club's face after making impact. Because of the high spin rate, amateur golfers may have a difficult time controlling the ball and hitting it in a relatively straight line. Such high-spin balls tend to have a side-spin so that when a golfer hook or slices the ball, it may drift off-course and land in a neighboring fairway.

Conversely, if the ball's mass is concentrated towards the outer surface, more force is required to change its rotational rate, and the ball has a relatively high Moment of Inertia. In such balls, the center piece (that is, the inner core) has a lower specific gravity than the outer piece (that is, the outer core layer). That is, in such balls, most of the mass is located away from the ball's axis of rotation and more force is needed to generate spin. Thus, the ball has a generally low spin rate as the ball leaves the club's face after making impact. Because of the low spin rate, amateur golfers may have an easier time controlling the ball and hitting it in a relatively straight line. The ball tends to travel a greater distance which is particularly important for driver shots off the tee.

As described in Sullivan, U.S. Pat. No. 6,494,795 and Ladd et al., U.S. Pat. No. 7,651,415, the formula for the Moment of Inertia for a sphere through any diameter is given in the CRC Standard Mathematical Tables, 24th Edition, 1976 at 20 (hereinafter CRC reference). In the present invention, the finished golf balls preferably have a Moment of Inertia in the range of about 55.0 g./cm<sup>2</sup> to about 95.0 g./cm<sup>2</sup>, preferably about 62.0 g./cm<sup>2</sup> to about 92.0 g./cm<sup>2</sup>.

The term, "specific gravity" as used herein, has its ordinary and customary meaning, that is, the ratio of the density of a substance to the density of water at 4° C., and the density of water at this temperature is 1 g/cm<sup>3</sup>.

The golf balls of this invention preferably have a high Moment of Inertia and are relatively low spin and long distance. The ball tends to travel a long distance and has less side-spin when a club face makes impact with the ball. The above-described core construction (wherein the inner core is made of a foamed composition and the surrounding outer core is preferably made of a thermoset rubber composition and the specific gravity of the outer core is greater than the specific gravity of the inner core [SG<sub>outer core</sub>>SG<sub>center</sub>]) contributes to the high MOI properties of the ball. Also, as discussed above, the rubber used to make the outer core may contain metal fillers, and these bits of mass are positioned away from the center of the ball. In addition, the outer surface of the inner core contains projecting members, thus providing additional mass that is positioned away from the center of the ball. Since most of the ball's mass is located away from the ball's center (axis of rotation), this helps produce high MOI properties. The resulting ball has relatively low spin and can relatively long distance properties.

The projecting members on the outer surface of the inner core also may help improve adhesion between the outer surface and composition of the outer core layer that will be applied over the inner core. By improving the adhesion, between these layers, the ball durability and ball speed also may be increased.

The foam cores and resulting balls also have relatively high resiliency so the ball will reach a relatively high velocity when struck by a golf club and travel a long distance. In particular, the inner foam cores of this invention preferably have a Coefficient of Restitution (COR) of about 0.300 or greater; more preferably about 0.400 or greater, and even more preferably about 0.450 or greater. The resulting balls containing the dual-layered core constructions of this invention and cover of at least one layer preferably have a COR of about 0.700 or greater, more preferably about 0.730 or greater; and even more preferably about 0.750 to 0.810 or greater.

The USGA has established a maximum weight of 45.93 g (1.62 ounces) for golf balls. For play outside of USGA rules, the golf balls can be heavier. In one preferred embodiment, the weight of the multi-layered core is in the range of about 28 to about 42 grams.

#### Cover Structure

The golf ball cores of this invention may be enclosed with one or more cover layers. In one version, the golf ball includes a multi-layered cover comprising inner and outer cover layers. The inner cover layer is preferably formed from a composition comprising an ionomer or a blend of two or more ionomers that helps impart hardness to the ball. In a particular embodiment, the inner cover layer is formed from a composition comprising a high acid ionomer. A particularly suitable high acid ionomer is Surlyn 8150® (DuPont). Surlyn 8150® is a copolymer of ethylene and methacrylic acid, having an acid content of 19 wt %, which is 45% neutralized with sodium. In another particular embodiment, the inner cover layer is formed from a composition comprising a high acid ionomer and a maleic anhydride-grafted non-ionomeric polymer. A particularly suitable maleic anhydride-grafted polymer is Fusabond 525D® (DuPont). Fusabond 525D® is a maleic anhydride-grafted, metallocene-catalyzed ethylene-butene copolymer having about 0.9 wt % maleic anhydride grafted onto the copolymer. A particularly preferred blend of high acid ionomer and maleic anhydride-grafted polymer is an 84 wt %/16 wt % blend of Surlyn 8150® and Fusabond 525D®. Blends of high acid ionomers with maleic anhydride-grafted polymers are further disclosed, for example, in U.S. Pat. Nos. 6,992,135 and 6,677,401, the entire disclosures of which are hereby incorporated herein by reference.

The inner cover layer also may be formed from a composition comprising a 50/45/5 blend of Surlyn® 8940/Surlyn® 9650/Nucrel® 960, and, in a particularly preferred embodiment, the composition has a material hardness of from 80 to 85 Shore C. In yet another version, the inner cover layer is formed from a composition comprising a 50/25/25 blend of Surlyn® 8940/Surlyn® 9650/Surlyn® 9910, preferably having a material hardness of about 90 Shore C. The inner cover layer also may be formed from a composition comprising a 50/50 blend of Surlyn® 8940/Surlyn® 9650, preferably having a material hardness of about 86 Shore C. A composition comprising a 50/50 blend of Surlyn® 8940 and Surlyn® 7940 also may be used. Surlyn® 8940 is an E/MAA copolymer in which the MAA acid groups have been partially neutralized with sodium ions. Surlyn® 9650 and Surlyn® 9910 are two different grades of E/MAA copolymer in which the MAA acid groups

have been partially neutralized with zinc ions. Nucrel® 960 is an E/MAA copolymer resin nominally made with 15 wt % methacrylic acid.

A wide variety of materials may be used for forming the outer cover including, for example, polyurethanes; polyureas; copolymers, blends and hybrids of polyurethane and polyurea; olefin-based copolymer ionomer resins (for example, Surlyn® ionomer resins and DuPont HPF® 1000 and HPF® 2000, commercially available from DuPont; 10 Iotek® ionomers, commercially available from ExxonMobil Chemical Company; Amplify® ionomers onomers of ethylene acrylic acid copolymers, commercially available from The Dow Chemical Company; and Clarix® ionomer resins, commercially available from A. Schulman Inc.); polyethylene, including, for example, low density polyethylene, linear low density polyethylene, and high density polyethylene; polypropylene; rubber-toughened olefin polymers; acid copolymers, for example, poly(meth)acrylic acid, which do not become part of an ionomeric copolymer; elastomers; 15 flexomers; styrene/butadiene/styrene block copolymers; styrene/ethylene-butylene/styrene block copolymers; dynamically vulcanized elastomers; copolymers of ethylene and vinyl acetates; copolymers of ethylene and methyl acrylates; polyvinyl chloride resins; polyamides, poly(amide-ester) 20 elastomers, and graft copolymers of ionomer and polyamide including, for example, Pebax® thermoplastic polyether block amides, commercially available from Arkema Inc; cross-linked trans-polyisoprene and blends thereof; polyester-based thermoplastic elastomers, such as Hytrel®, commercially available from DuPont or RiteFlex®, commercially available from Ticona Engineering Polymers; polyurethane-based thermoplastic elastomers, such as Elastollan®, commercially available from BASF; synthetic or natural vulcanized rubber; and combinations thereof. 25 30 35 Castable polyurethanes, polyureas, and hybrids of polyurethanes-polyureas are particularly desirable because these materials can be used to make a golf ball having high resiliency and a soft feel. By the term, "hybrids of polyurethane and polyurea," it is meant to include copolymers and blends thereof.

Polyurethanes, polyureas, and blends, copolymers, and hybrids of polyurethane/polyurea are also particularly suitable for forming cover layers. When used as cover layer materials, polyurethanes and polyureas can be thermoset or thermoplastic. Thermoset materials can be formed into golf ball layers by conventional casting or reaction injection molding techniques. Thermoplastic materials can be formed into golf ball layers by conventional compression or injection molding techniques.

50 The inner cover layer preferably has a material hardness within a range having a lower limit of 70 or 75 or 80 or 82 Shore C and an upper limit of 85 or 86 or 90 or 92 Shore C. The thickness of the inner cover layer is preferably within a range having a lower limit of 0.010 or 0.015 or 0.020 or 0.030 inches and an upper limit of 0.035 or 0.045 or 0.080 or 0.120 inches. The outer cover layer preferably has a material hardness of 85 Shore C or less. The thickness of the outer cover layer is preferably within a range having a lower limit of 0.010 or 0.015 or 0.025 inches and an upper limit of 0.035 or 0.040 or 0.055 or 0.080 inches. Methods for measuring hardness of the layers in the golf ball are described in further detail below.

55 60 65 As discussed above, the core structure of this invention may be enclosed with one or more cover layers. In one embodiment, a multi-layered cover comprising inner and outer cover layers is formed, where the inner cover layer has a thickness of about 0.01 inches to about 0.06 inches, more

preferably about 0.015 inches to about 0.040 inches, and most preferably about 0.02 inches to about 0.035 inches. In this version, the inner cover layer is formed from a partially- or fully-neutralized ionomer having a Shore D hardness of greater than about 55, more preferably greater than about 60, and most preferably greater than about 65. The outer cover layer, in this embodiment, preferably has a thickness of about 0.015 inches to about 0.055 inches, more preferably about 0.02 inches to about 0.04 inches, and most preferably about 0.025 inches to about 0.035 inches, with a hardness of about Shore D 80 or less, more preferably 70 or less, and most preferably about 60 or less. The inner cover layer is harder than the outer cover layer in this version. A preferred outer cover layer is a castable or reaction injection molded polyurethane, polyurea or copolymer, blend, or hybrid thereof having a Shore D hardness of about 40 to about 50. In another multi-layer cover, dual-core embodiment, the outer cover and inner cover layer materials and thickness are the same but, the hardness range is reversed, that is, the outer cover layer is harder than the inner cover layer. For this harder outer cover/softer inner cover embodiment, the ionomer resins described above would preferably be used as outer cover material.

#### Golf Ball Construction

The solid cores for the golf balls of this invention may be made using any suitable conventional technique such as, for example, compression or injection molding. In some embodiments, the inner core is formed by compression molding a slug of the uncured or lightly cured polybutadiene rubber material into a substantially spherical structure. In other embodiments, inner cores having non-spherical structures are made. For example, the outer surface of the inner core may have non-uniform thickness and contain ribs, ridges, bumps, nubs, spines, and other projecting members. The intermediate and outer core layers, which surround the inner core, are formed by molding compositions over the inner core. Compression or injection molding techniques may be used. Then, the intermediate (casing) and/or cover layers are applied. Prior to this step, the core structure may be surface-treated to increase the adhesion between its outer surface and the next layer that will be applied over the core. Such surface-treatment may include mechanically or chemically-abrading the outer surface of the core. For example, the core may be subjected to corona-discharge, plasma-treatment, silane-dipping, or other treatment methods known to those in the art.

The cover layers are formed over the core or ball subassembly (the core structure and any casing layers disposed about the core) using a suitable technique such as, for example, compression-molding, flip-molding, injection-molding, retractable pin injection-molding, reaction injection-molding (RIM), liquid injection-molding, casting, spraying, powder-coating, vacuum-forming, flow-coating, dipping, spin-coating, and the like. Preferably, each cover layer is separately formed over the ball subassembly. For example, an ethylene acid copolymer ionomer composition may be injection-molded to produce half-shells. Alternatively, the ionomer composition can be placed into a compression mold and molded under sufficient pressure, temperature, and time to produce the hemispherical shells. The smooth-surfaced hemispherical shells are then placed around the ball subassembly in a compression mold. Under sufficient heating and pressure, the shells fuse together to form an inner cover layer that surrounds the subassembly. In another method, the ionomer composition is injection-molded directly onto the core using retractable pin injection

molding. An outer cover layer comprising a polyurethane or polyurea composition may be formed by using a casting process.

For example, in one version of the casting process, a liquid mixture of reactive polyurethane prepolymer and chain-extender (curing agent) is poured into lower and upper mold cavities. Then, the golf ball subassembly is lowered at a controlled speed into the reactive mixture. Ball suction cups can hold the ball subassembly in place via reduced pressure or partial vacuum. After sufficient gelling of the reactive mixture (typically about 4 to about 12 seconds), the vacuum is removed and the intermediate ball is released into the mold cavity. Then, the upper mold cavity is mated with the lower mold cavity under sufficient pressure and heat. An exothermic reaction occurs when the polyurethane prepolymer and chain extender are mixed and this continues until the cover material encapsulates and solidifies around the ball subassembly. Finally, the molded balls are cooled in the mold and removed when the molded cover is hard enough so that it can be handled without deformation.

After the golf balls have been removed from the mold, they may be subjected to finishing steps such as flash-trimming, surface-treatment, marking, coating, and the like using techniques known in the art. For example, in traditional white-colored golf balls, the white-pigmented cover may be surface-treated using a suitable method such as, for example, corona, plasma, or ultraviolet (UV) light-treatment. Then, indicia such as trademarks, symbols, logos, letters, and the like may be printed on the ball's cover using pad-printing, ink-jet printing, dye-sublimation, or other suitable printing methods. Clear surface coatings (for example, primer and top-coats), which may contain a fluorescent whitening agent, are applied to the cover. The resulting golf ball has a glossy and durable surface finish.

In another finishing process, the golf balls are painted with one or more paint coatings. For example, white primer paint may be applied first to the surface of the ball and then a white top-coat of paint may be applied over the primer. Of course, the golf ball may be painted with other colors, for example, red, blue, orange, and yellow. As noted above, markings such as trademarks and logos may be applied to the painted cover of the golf ball. Finally, a clear surface coating may be applied to the cover to provide a shiny appearance and protect any logos and other markings printed on the ball.

Different ball constructions can be made using the different core constructions of this invention as shown in FIGS. 1-15 discussed above. Such golf ball designs include, for example, three-piece, four-piece, five-piece, and six-piece designs. It should be understood that the core constructions and golf balls shown in FIGS. 1-15 are for illustrative purposes only and are not meant to be restrictive. Other core constructions and golf balls can be made in accordance with this invention.

For example, a multi-layered core structure having an inner core (center); intermediate core layer; and outer core layer can be made. A cover having a single or multiple layers may be disposed about the multi-layered core. The inner core layer may comprise a foamed composition, such as polyurethane foam, as discussed above. The intermediate and outer core layers may be made of thermoset or thermoplastic compositions. Each of the core layers may have a positive hardness gradient, and there may be a positive hardness gradient across the entire core assembly. In such a core construction, the specific gravity of the outer core ( $SG_{outer}$ ) is preferably greater than the specific gravity of the

intermediate core layer ( $SG_{intermediate}$ ); and the  $SG_{intermediate}$  is greater than the specific gravity of the foamed inner core layer ( $SG_{inner}$ ).

#### Test Methods

##### Hardness.

The center hardness of a core is obtained according to the following procedure. The core is gently pressed into a hemispherical holder having an internal diameter approximately slightly smaller than the diameter of the core, such that the core is held in place in the hemispherical portion of the holder while concurrently leaving the geometric central plane of the core exposed. The core is secured in the holder by friction, such that it will not move during the cutting and grinding steps, but the friction is not so excessive that distortion of the natural shape of the core would result. The core is secured such that the parting line of the core is roughly parallel to the top of the holder. The diameter of the core is measured 90 degrees to this orientation prior to securing. A measurement is also made from the bottom of the holder to the top of the core to provide a reference point for future calculations. A rough cut is made slightly above the exposed geometric center of the core using a band saw or other appropriate cutting tool, making sure that the core does not move in the holder during this step. The remainder of the core, still in the holder, is secured to the base plate of a surface grinding machine. The exposed 'rough' surface is ground to a smooth, flat surface, revealing the geometric center of the core, which can be verified by measuring the height from the bottom of the holder to the exposed surface of the core, making sure that exactly half of the original height of the core, as measured above, has been removed to within 0.004 inches. Leaving the core in the holder, the center of the core is found with a center square and carefully marked and the hardness is measured at the center mark according to ASTM D-2240. Additional hardness measurements at any distance from the center of the core can then be made by drawing a line radially outward from the center mark, and measuring the hardness at any given distance along the line, typically in 2 mm increments from the center. The hardness at a particular distance from the center should be measured along at least two, preferably four, radial arms located 180° apart, or 90° apart, respectively, and then averaged. All hardness measurements performed on a plane passing through the geometric center are performed while the core is still in the holder and without having disturbed its orientation, such that the test surface is constantly parallel to the bottom of the holder, and thus also parallel to the properly aligned foot of the durometer.

The outer surface hardness of a golf ball layer is measured on the actual outer surface of the layer and is obtained from the average of a number of measurements taken from opposing hemispheres, taking care to avoid making measurements on the parting line of the core or on surface defects, such as holes or protrusions. Hardness measurements are made pursuant to ASTM D-2240 "Indentation Hardness of Rubber and Plastic by Means of a Durometer." Because of the curved surface, care must be taken to ensure that the golf ball or golf ball sub-assembly is centered under the durometer indenter before a surface hardness reading is obtained. A calibrated, digital durometer, capable of reading to 0.1 hardness units is used for the hardness measurements. The digital durometer must be attached to, and its foot made parallel to, the base of an automatic stand. The weight on the durometer and attack rate conforms to ASTM D-2240.

In certain embodiments, a point or plurality of points measured along the "positive" or "negative" gradients may be above or below a line fit through the gradient and its

outermost and innermost hardness values. In an alternative preferred embodiment, the hardest point along a particular steep "positive" or "negative" gradient may be higher than the value at the innermost portion of the inner core (the geometric center) or outer core layer (the inner surface)—as long as the outermost point (i.e., the outer surface of the inner core) is greater than (for "positive") or lower than (for "negative") the innermost point (i.e., the geometric center of the inner core or the inner surface of the outer core layer), such that the "positive" and "negative" gradients remain intact.

As discussed above, the direction of the hardness gradient of a golf ball layer is defined by the difference in hardness measurements taken at the outer and inner surfaces of a particular layer. The center hardness of an inner core and hardness of the outer surface of an inner core in a single-core ball or outer core layer are readily determined according to the test procedures provided above. The outer surface of the inner core layer (or other optional intermediate core layers) in a dual-core ball are also readily determined according to the procedures given herein for measuring the outer surface hardness of a golf ball layer, if the measurement is made prior to surrounding the layer with an additional core layer. Once an additional core layer surrounds a layer of interest, the hardness of the inner and outer surfaces of any inner or intermediate layers can be difficult to determine. Therefore, for purposes of the present invention, when the hardness of the inner or outer surface of a core layer is needed after the inner layer has been surrounded with another core layer, the test procedure described above for measuring a point located 1 mm from an interface is used. Likewise, the midpoint of a core layer is taken at a point equidistant from the inner surface and outer surface of the layer to be measured, most typically an outer core layer. As noted above, once one or more core layers surround a layer of interest, the exact midpoint may be difficult to determine, therefore, for the purposes of the present invention, the measurement of "midpoint" hardness of a layer is taken within plus or minus 1 mm of the measured midpoint of the layer.

Also, it should be understood that there is a fundamental difference between "material hardness" and "hardness as measured directly on a golf ball." For purposes of the present invention, material hardness is measured according to ASTM D2240 and generally involves measuring the hardness of a flat "slab" or "button" formed of the material. Surface hardness as measured directly on a golf ball (or other spherical surface) typically results in a different hardness value. The difference in "surface hardness" and "material hardness" values is due to several factors including, but not limited to, ball construction (that is, core type, number of cores and/or cover layers, and the like); ball (or sphere) diameter; and the material composition of adjacent layers. It also should be understood that the two measurement techniques are not linearly related and, therefore, one hardness value cannot easily be correlated to the other. Shore hardness (for example, Shore C or Shore D hardness) was measured according to the test method ASTM D-2240.

#### Compression.

As disclosed in Jeff Dalton's *Compression by Any Other Name, Science and Golf IV, Proceedings of the World Scientific Congress of Golf* (Eric Thain ed., Routledge, 2002) ("J. Dalton"), several different methods can be used to measure compression, including Atti compression, Riehle compression, load/deflection measurements at a variety of fixed loads and offsets, and effective modulus. For purposes of the present invention, "compression" refers to Atti compression and is measured according to a known procedure,

using an Atti compression test device, wherein a piston is used to compress a ball against a spring. The travel of the piston is fixed and the deflection of the spring is measured. The measurement of the deflection of the spring does not begin with its contact with the ball; rather, there is an offset of approximately the first 1.25 mm (0.05 inches) of the spring's deflection. Very low stiffness cores will not cause the spring to deflect by more than 1.25 mm and therefore have a zero compression measurement. The Atti compression tester is designed to measure objects having a diameter of 42.7 mm (1.68 inches); thus, smaller objects, such as golf ball cores, must be shimmed to a total height of 42.7 mm to obtain an accurate reading. Conversion from Atti compression to Riehle (cores), Riehle (balls), 100 kg deflection, 130-10 kg deflection or effective modulus can be carried out according to the formulas given in J. Dalton. Compression may be measured as described in McNamara et al., U.S. Pat. No. 7,777,871, the disclosure of which is hereby incorporated by reference.

#### Drop Rebound.

By "drop rebound," it is meant the number of inches a sphere will rebound when dropped from a height of 72 inches in this case, measuring from the bottom of the sphere. A scale, in inches is mounted directly behind the path of the dropped sphere and the sphere is dropped onto a heavy, hard base such as a slab of marble or granite (typically about 1 ft wide by 1 ft high by 1 ft deep). The test is carried out at about 72-75° F. and about 50% RH.

#### Coefficient of Restitution ("COR").

The COR is determined according to a known procedure, wherein a golf ball or golf ball subassembly (for example, a golf ball core) is fired from an air cannon at two given velocities and a velocity of 125 ft/s is used for the calculations. Ballistic light screens are located between the air cannon and steel plate at a fixed distance to measure ball velocity. As the ball travels toward the steel plate, it activates each light screen and the ball's time period at each light screen is measured. This provides an incoming transit time period which is inversely proportional to the ball's incoming velocity. The ball makes impact with the steel plate and rebounds so it passes again through the light screens. As the rebounding ball activates each light screen, the ball's time period at each screen is measured. This provides an outgoing transit time period which is inversely proportional to the ball's outgoing velocity. The COR is then calculated as the ratio of the ball's outgoing transit time period to the ball's incoming transit time period (COR=V<sub>out</sub>/V<sub>in</sub>=T<sub>in</sub>/T<sub>out</sub>).

#### Examples

In the following Examples, different foam formulations were used to prepare core samples using the above-described molding methods. The different formulations are described in Tables 1 and 2 below.

TABLE 1

| Ingredient                                            | Weight Percent |
|-------------------------------------------------------|----------------|
| 4,4 Methylene Diphenyl Diisocyanate (MDI)             | 14.65%         |
| Polytetramethylene ether glycol (PTMEG 2000)          | 34.92%         |
| *Mondur™ 582 (2.5 fn)                                 | 29.11%         |
| Trifunctional caprolactone polyol (CAPA 3031 (3.0 fn) | 20.22%         |

TABLE 1-continued

| (Sample A)                   |                |
|------------------------------|----------------|
| Ingredient                   | Weight Percent |
| Water                        | 0.67%          |
| **Niax™ L-1500 surfactant    | 0.04%          |
| *** KKAT™ XK 614 catalyst    | 0.40%          |
| Dibutyl tin dilaurate (T-12) | 0.03%          |

10 \*Mondur™ 582 (2.5 fn) - polymeric methylene diphenyl diisocyanate (p-MDI) with 2.5 functionality, available from Bayer Material Science.  
 \*\*Niax™ L-1500 silicone-based surfactant, available from Momentive Specialty Chemicals, Inc.  
 \*\*\* KKAT™ XK 614 zinc-based catalyst, available from King Industries.

15 The resulting spherical core Sample A (0.75 inch diameter) had a density of 0.45 g/cm<sup>3</sup>, a compression (SCDI) of 75, and drop rebound of 46% based on average measurements using the test methods as described above.

TABLE 2

| (Sample B)                   |                |
|------------------------------|----------------|
| Ingredient                   | Weight Percent |
| Mondur™ 582 (2.5 fn)         | 30.35%         |
| *Desmodur™ 3900 aliphatic    | 30.35%         |
| **Polymeg™ 650               | 19.43%         |
| ***Ethacure™ 300             | 19.43%         |
| Water                        | 0.31%          |
| Niax™ L-1500 surfactant      | 0.04%          |
| Dibutyl tin dilaurate (T-12) | 0.09%          |

30 \*Desmodur™ 3900 - polyfunctional aliphatic polyisocyanate resin based on hexamethylene diisocyanate (HDI), available from Bayer Material Science.  
 \*\*Polymeg™ 650 - polytetramethylene ether glycol, available from Lyondell Chemical Company.  
 \*\*\*Ethacure™ 300 - aromatic diamine curing agent, available from Albemarle Corp.

35 The resulting spherical core Sample B (0.75 inch diameter) had a density of 0.61 g/cm<sup>3</sup>, a compression (SCDI) of 160, and drop rebound of 56% based on average measurements using the test methods as described above.

40 When numerical lower limits and numerical upper limits are set forth herein, it is contemplated that any combination of these values may be used. Other than in the operating examples, or unless otherwise expressly specified, all of the numerical ranges, amounts, values and percentages such as those for amounts of materials and others in the specification may be read as if prefaced by the word "about" even though the term "about" may not expressly appear with the value, amount or range. Accordingly, unless indicated to the contrary, the numerical parameters set forth in the specification and attached claims are approximations that may vary depending upon the desired properties sought to be obtained by the present invention.

45 All patents, publications, test procedures, and other references cited herein, including priority documents, are fully incorporated by reference to the extent such disclosure is not inconsistent with this invention and for all jurisdictions in which such incorporation is permitted. It is understood that the compositions, golf ball components, and finished golf balls described and illustrated herein represent only some embodiments of the invention. It is appreciated by those skilled in the art that various changes and additions can be made to compositions and products without departing from the spirit and scope of this invention. It is intended that all such embodiments be covered by the appended claims.

50 65 We claim:

1. A golf ball, comprising a multi-layered core assembly and a cover, the core assembly comprising:

- i) an inner core comprising a foamed polyurethane, the inner core having a center and outer surface, and a diameter in the range of about 0.100 to about 1.100 inches, the inner core having a specific gravity ( $SG_{inner}$ ) and projecting members on the outer surface;
  - ii) an intermediate core layer comprising a non-foamed thermoset or thermoplastic material, the intermediate core having a specific gravity ( $SG_{intermediate}$ ); and
  - iii) an outer core layer comprising a non-foamed thermoset or thermoplastic material, the outer core layer being disposed about the inner core and having a thickness in the range of about 0.200 to about 0.800 inches, the outer core having a specific gravity ( $SG_{outer}$ ), wherein the  $SG_{outer}$  is greater than the  $SG_{intermediate}$  and the  $SG_{intermediate}$  is greater than the  $SG_{inner}$ ; and
- the cover comprising at least one layer disposed about the multi-layered core assembly.

2. The golf ball of claim 1, wherein at least one of the intermediate and outer core layers comprises a thermoset rubber selected from the group consisting of polybutadiene, ethylene-propylene rubber, ethylene-propylene-diene rubber, polyisoprene, styrene-butadiene rubber, polyalkenamers, and butyl rubber, and mixtures thereof.

3. The golf ball of claim 2, wherein the thermoset rubber is polybutadiene rubber.

4. The golf ball of claim 1, wherein at least one of the intermediate and outer core layers comprises a thermoplastic polymer selected from the group consisting of partially-neutralized ionomers; highly-neutralized ionomers; polyesters; polyamides; polyamide-ethers, polyamide-esters; polyurethanes, polyureas; fluoropolymers; polystyrenes; polypropylenes; polyethylenes; polyvinyl chlorides; polyvinyl acetates; polycarbonates; polyvinyl alcohols; polyester-ethers; polyethers; polyimides, polyetherketones, polyamidemides; and mixtures thereof.

5. The golf ball of claim 4, wherein the thermoplastic material is an ionomer composition comprising an O/X-type copolymer, wherein O is selected from the group consisting of ethylene and propylene, and X is selected from the group consisting of methacrylic acid, acrylic acid, ethacrylic acid, crotonic acid, maleic acid, fumaric acid, and itaconic acid.

6. The golf ball of claim 1, wherein the cover is a single layer having a thickness of about 0.015 to about 0.090 inches and is formed from a thermoplastic or thermoset material.

7. The golf ball of claim 1, wherein the cover comprises an inner cover layer and outer cover layer, each cover having a surface hardness, wherein the surface hardness of the inner cover layer is greater than the surface hardness of the outer cover layer.

8. The golf ball of claim 1, wherein the projecting members of the inner core are spaced apart from each other and gaps are located between the projections.

9. The golf ball of claim 8, wherein the projecting members are shaped and positioned so that the inner core has a substantially spherical shape.

10. The golf ball of claim 1, wherein the inner core has a center hardness ( $H_{inner\ core\ center}$ ), and the outer core has an outer surface hardness ( $H_{outer\ surface\ of\ OC}$ ), the  $H_{inner\ core\ center}$  being in the range of about 10 to about 80 Shore C and the  $H_{outer\ surface\ of\ OC}$  being in the range of about 65 to about 96 Shore C to provide a positive hardness gradient across the core assembly.

11. A golf ball, comprising a multi-layered core assembly, and intermediate layer, and a cover, the core assembly comprising:

- i) an inner core comprising a foamed polyurethane, the inner core having a center and outer surface, and a diameter in the range of about 0.100 to about 1.100 inches, the inner core having a specific gravity ( $SG_{inner}$ ) and projecting members on the outer surface;
- ii) an intermediate core layer comprising a non-foamed thermoset or thermoplastic material, the intermediate core having a specific gravity ( $SG_{intermediate}$ ); and
- iii) an outer core layer comprising a non-foamed thermoset or thermoplastic material, the outer core layer being disposed about the inner core and having a thickness in the range of about 0.200 to about 0.800 inches, the outer core having a specific gravity ( $SG_{outer}$ ), wherein the  $SG_{outer}$  is greater than the  $SG_{intermediate}$  and the  $SG_{intermediate}$  is greater than the  $SG_{inner}$ ; and

a cover comprising at least one layer, and a casing layer, the casing layer being disposed between the core assembly and cover.

12. The golf ball of claim 11, wherein the casing layer comprises a thermoplastic polymer selected from the group consisting of partially-neutralized ionomers; highly-neutralized ionomers; polyesters; polyamides; polyamide-ethers, polyamide-esters; polyurethanes, polyureas; fluoropolymers; polystyrenes; polypropylenes; polyethylenes; polyvinyl chlorides; polyvinyl acetates; polycarbonates; polyvinyl alcohols; polyester-ethers; polyethers; polyimides, polyetherketones, polyamidemides; and mixtures thereof.

13. The golf ball of claim 11, wherein the thermoplastic material is an ionomer composition comprising an O/X-type copolymer, wherein O is selected from the group consisting of ethylene and propylene, and X is selected from the group consisting of methacrylic acid, acrylic acid, ethacrylic acid, crotonic acid, maleic acid, fumaric acid, and itaconic acid.

14. The golf ball of claim 13, wherein the O of the O/X-type acid copolymer is ethylene and the X is methacrylic acid or acrylic acid.

15. The golf ball of claim 13, wherein the O/X-type acid copolymer contains acid groups and 30 to 70% of the acid groups are neutralized.

16. The golf ball of claim 13, wherein the O/X-type acid copolymer contains acid groups and greater than 70% of the acid groups are neutralized.

17. The golf ball of claim 13, wherein the ionomer composition further comprises fatty acids or salts of fatty acids.